

Jan. 16, 1968

C. R. BARR

3,364,022

DIRECT POSITIVE PHOTOGRAPHIC COLOR REPRODUCTION PROCESS AND  
ELEMENT UTILIZING THIO-SUBSTITUTED HYDROQUINONES  
AS DEVELOPMENT INHIBITORS  
Filed Dec. 1, 1966

Fig. 1



Fig. 2



CHARLES R. BARR

INVENTOR

BY *James R. Furlent*  
*Ogden H. Webster*

ATTORNEYS

1

3,364,022  
**DIRECT POSITIVE PHOTOGRAPHIC COLOR REPRODUCTION PROCESS AND ELEMENT UTILIZING THIO-SUBSTITUTED HYDROQUINONES AS DEVELOPMENT INHIBITORS**

Charles R. Barr, Rochester, N.Y., assignor to Eastman Kodak Company, Rochester, N.Y., a corporation of New Jersey

Continuation-in-part of application Ser. No. 412,591, Nov. 16, 1964, which is a continuation-in-part of application Ser. No. 269,346, Apr. 1, 1963. This application Dec. 1, 1966, Ser. No. 598,480

25 Claims. (Cl. 96—3)

## ABSTRACT OF THE DISCLOSURE

Photographic direct positive color elements and processes feature a non-diffusible thio-substituted hydroquinone which reacts with oxidized developing agent to form a diffusible mercaptan development inhibitor. This mercaptan diffuses to a predetermined layer of the photographic element and selectively inhibits development of color former present therein.

This application is a continuation-in-part application of our copending application U.S. Ser. No. 412,591, filed Nov. 16, 1964, now abandoned; which is a continuation-in-part application of our U.S. application Ser. No. 269,346; filed Apr. 1, 1963, now abandoned.

This invention relates to color photography, and more particularly to photographic direct positive color processes and photographic elements suitable for use in such processes.

Direct positive photographic color processes are well known in the art and generally comprise a number of steps. A typical color process comprises such steps as a black-and-white development to form a negative image, a reversal exposure, development with an aromatic primary amino color developing agent to form insoluble image dyes in the areas of development, and a bleach step to remove developed silver. Color processes are also known whereby color images are transferred to receiving elements and which have the advantage of producing color images free of residual color couplers and other products of development. However, many of such processes of both types involve several complex steps and require several processing baths with large volumes of processing solutions.

It is an object of the present invention to provide a new color process in the photographic art.

It is another object of this invention to provide a new photographic process for producing sharp color images.

It is a further object of this invention to provide a novel photographic diffusion transfer process wherein a dye image is transferred to a receiving layer.

It is another object of this invention to provide a novel color diffusion transfer process that can be effected in one wet processing step.

It is an additional object of this invention to provide a novel color diffusion transfer process wherein the color development is carried out in the presence of a predominant proportion of the products of oxidation of the color developing agent.

It is still another object of this invention to provide a novel process for preparing direct positive color images.

It is also an object of this invention to provide a novel color diffusion transfer process for producing direct positive full-color images.

It is likewise an object of this invention to provide a novel photographic element suitable for use in preparing

2

direct positive color images by a photographic diffusion transfer process.

These and other objects are attained by means of this invention as described hereinafter with reference to preferred embodiments thereof.

The present invention concerns light-sensitive photographic elements having coated thereon at least two Color-Forming Units as described herein and which elements can be processed in the presence of alkaline color developing solutions containing aromatic primary amino color developing agents to prepare direct positive color images.

The Color-Forming Units of the invention comprise:

*Component A.*—A hydrophilic colloid-silver halide emulsion capable of recording latent images on exposure to light;

*Component B.*—A nondiffusible hydrophilic hydroquinone compound capable of releasing a diffusible mercaptan development inhibitor when the hydroquinone cross-20 oxidizes with oxidized color developer, such development inhibitor releasing hydroquinones being referred herein as DIR compounds. This "DIR" compound is utilized in the color forming unit;

*Component C.*—An emulsion of a hydrophilic colloid and a water-insoluble metal salt developable to substantial density without exposure to light, and which is referred to herein as a "spontaneously" developable" emulsion;

*Component D.*—A nondiffusible photographic color coupler capable of forming a diffusible acid dye on development with an alkaline color developing solution containing an aromatic primary amino color developing agent, and which diffusible-dye-releasing coupler is referred to herein as a "DDR" coupler;

*Component D'.*—A nondiffusible photographic color coupler capable of forming a nondiffusible dye on development with an alkaline color developing solution containing an aromatic primary amino color developing agent.

When such Color-Forming Units are exposed, a latent image (negative image) pattern of developable silver halide is formed in the light-sensitive emulsion (Component A). When this exposed emulsion is developed in an alkaline color developing solution containing an aromatic primary amino color developing agent in the presence of a DIR compound (Component B), the DIR compound reacts with color development oxidation product to release a diffusible mercaptan development inhibitor. The resulting diffusible development inhibitor diffuses image-wise to the "spontaneously" developable emulsion (Component C) inhibiting development in regions corresponding to the latent image pattern (negative image area) formed in the light-sensitive emulsion. A coupler<sup>1</sup> (Component D or D') is contiguous to the developable metal salt of the "spontaneously" developable emulsion. The developable metal salt of the "spontaneously" developable emulsion in regions not inhibited against development by the diffusible development inhibitor (positive image area) develops and a dye image is formed in such regions when the coupler reacts with color development oxidation product. When DDR couplers are used (Component D), the resulting acid dye diffuses image-wise in register to a juxtaposed reception layer containing a mordant for acid dyes to produce a positive color reproduction. When conventional couplers are used (Component D'), the resulting image dyes are non-diffusible and remain in the photoelement. This photoelement must then be bleached and fixed to remove the developed silver and residual silver halide, thus leaving only the non-diffusible dye image.

<sup>1</sup> I.e. either DDR type or conventional type.

The Color-Forming Units are prepared so that the light sensitive emulsion develops and a development inhibitor is released from the DIR compound a finite time prior to the development of the "spontaneously" developable emulsion and the subsequent formation of the image dye. Such can be accomplished by physically disposing the light-sensitive emulsion (Component A) and the contiguous DIR compound (Component B) further from the support than the "spontaneously" developable emulsion, by utilizing a silver halide emulsion having a shorter development induction period for the light-sensitive emulsion than the developable metal salt in the "spontaneously" developable emulsion, and/or by utilizing DIR compounds that react at a faster rate than the couplers.

The couplers and DIR compounds are integral components of the present elements. The DIR compounds can be incorporated either in, or in a layer contiguous to, the light sensitive emulsion, and the coupler (DDR or conventional type) can be incorporated either in, or in a layer contiguous to, the "spontaneously" developable emulsion.

Photographic elements suitable for preparing correct full-color positive renditions can be prepared by utilizing three of the present Color-Forming Units wherein the light sensitive emulsions are sensitive to red, green and blue light respectively, and the couplers capable of forming dyes complementary to the color of the spectral sensitivity of the respective Color-Forming Units. However, false sensitization can also be utilized in preparing the present photographic elements.

The DDR or diffusible-dye-releasing couplers used in the photographic elements of the invention are initially nondiffusing in the layers of the element but form dyes diffusible in the layers of the element on reaction with oxidation products of aromatic primary amino silver halide photographic color developing agents. Such DDR couplers include those having the formulas:

DYE-LINK-(COUP-BALL)<sub>n</sub>

and

BALL-LINK-(COUP-SOL)<sub>n</sub>

BALL-LINK-COUP

wherein

(1) DYE is a dye radical containing an acidic solubilizing radical;

(2) LINK is a connecting or linkage radical such as azo ( $-\text{N}=\text{N}-$ ), azoxy



mercuri ( $-\text{Hg}-$ ), oxy ( $-\text{O}-$ ), alkylidene (includes both  $>\text{CH}-$  and  $=\text{CH}-$ ), monothio ( $-\text{S}-$ ) or dithio ( $-\text{S}-\text{S}-$ );

(3) COUP is a photographic color coupler radical such as a 5-pyrazolone coupler radical, a phenolic coupler radical or an open-chain ketomethylene coupler radical, the coupler radical being substituted in the coupling position with the connecting or linkage radical;

(4) BALL is a photographically inert organic radical of such molecular size and configuration as to render the coupler nondiffusing in the element in the alkaline color developing solution;

(5) SOL is either a hydrogen atom or an acidic solubilizing group when the color developing agent contains an acidic solubilizing radical, SOL always being an acidic solubilizing radical when the color developing agent is free of an acidic solubilizing group; and

(6)  $n$  is an integer of 1 or 2 when LINK is an alkylidene radical, and  $n$  is always 1 when LINK is one of the other aforementioned connecting radicals, namely, azo, azoxy, mercuri, oxy, thio, or dithio.

The acidic solubilizing radicals described above can be attached to the coupler and/or developer moieties of the dyes, and render the dyes diffusible in the element in alkaline processing solutions. Typical of such radicals

are carboxylic, sulfonic, ionizable sulfonamido, and hydroxy-substituted groups that lend to dyes negative charges.

Typical dye radical substituents (DYE) of the DDR couplers include azo, azomethine, indoaniline, indophenol, anthraquinone and related dye radicals well known in the art that exhibit selective absorption in the visible spectrum. The dye radicals contain acidic solubilizing moieties.

When DDR couplers having the formula DYE-LINK-(COUP-BALL)<sub>n</sub> as described above are reacted with oxidized color developing agent, the connecting radical (LINK) is split from the coupler moiety and a diffusible preformed acid dye (DYE) is released which diffuses imagewise to a reception layer. An acidic solubilizing group on the preformed dye lends diffusibility and mordantability to the dye molecule. The coupling portion of the DDR coupler (COUP) couples with color developing agent oxidation product to form a dye that is nondiffusible in the element because of the attached ballasting group (BALL) in a noncoupling position. In this type of DDR coupler, the color of the diffusible dye is determined by the color of the preformed dye moiety (DYE), the color of the reaction product of color developer oxidation product and the coupler moiety (COUP) being unimportant to the color of the diffusible image.

When DDR couplers having formula BALL-LINK-(COUP-SOL)<sub>n</sub> as described above are reacted with oxidized color developing agent, the connecting radical (LINK) is split from the coupler moiety and a diffusible dye is formed with the color developing agent oxidation product and the coupling portion (COUP) of the DDR coupler, which dye diffuses imagewise to a reception layer. Diffusibility is imparted to the dye by an acidic solubilizing group attached to a noncoupling position of the coupling portion (COUP) of the DDR coupler and/or to the color developing agent. The ballast portion of the DDR coupler remains immobile. In this type of DDR coupler, the color of the diffusible dye is determined by the color of the reaction product of color developer oxidation product and the coupler moiety (COUP).

When the coupler radical (COUP) in the DDR couplers is a 5-pyrazolone radical, we prefer to have substituted in the 3-position of the pyrazolone moiety an anilino group or an alkoxy group. When the coupler radical (COUP) in the DDR couplers is a cyan-forming phenolic coupler radical, we prefer to have substituted in the ortho or 2-position of the phenolic moiety a fully substituted amido group (e.g.,



wherein R is an alkyl group or a phenyl group). Also, when the connecting radical (LINK) in the DDR couplers having the formula, BALL-LINK-(COUP-SOL)<sub>n</sub>, is an azo radical, we prefer that the ballasting radical (BALL) be a phenyl radical containing either a hydroxy group or an amino group ( $-\text{NH}_2$ ) substituted in the ortho or 2-position of the phenyl moiety.

Typical conventional cyan, magenta and yellow forming couplers useful in this invention to form non-diffusible dyes on coupling with oxidation products of color developing agents may be found, for example, in the following U.S. patents:

65 Cyan: 2,895,826, Salminen et al., July 21, 1959; 2,474,293, Weissburger et al., June 28, 1949; 2,908,573, 2,908,573, Bush et al., October 13, 1959.

Magenta: 2,600,788, Loria et al., June 17, 1952; 2,908,573, Bush et al., October 13, 1959.

Yellow: 2,875,057, McCrossen et al., February 24, 1959; 2,908,573, Bush et al., October 13, 1959.

These non-diffusible-dye-forming couplers are represented by the following formula: BALL-COUP wherein BALL and COUP are as defined above and BALL is attached to the coupler in a non-coupling position.

Non-diffusible couplers of the formula BALL-LINK-COUP can be used when the color developing agent is supplied with a solubilizing function.

The DIR, development inhibitor releasing, hydroquinone compounds used in the photographic elements of the invention release development inhibiting mercaptans that are diffusible in the layers of the Color-Forming Unit. It is believed that the DIR hydroquinone compound cross-oxidizes with the oxidation product of aromatic primary amino silver halide developing agents. As a result of this cross-oxidation reaction, the hydroquinone is oxidized to the corresponding quinone. It is from this quinone only that the diffusible development inhibiting mercaptan is split.

The DIR compounds of this invention are non-diffusible, or ballasted, thio-substituted hydroquinones which react with oxidized color developing agent to form a diffusible mercaptan development inhibitor. If desired, thio-substituted hydroquinone compounds of this invention can be masked with an alkaline splittable group. That is, one or both of the hydroxyl groups of the hydroquinone can be replaced with any suitable substituent, such as an acyl group, which splits off under alkaline conditions to regenerate the hydroxyl group. A masking group inactivates a hydroxyl group of the hydroquinone compound. Masked hydroquinone compounds can be incorporated directly in light sensitive silver halide systems. Typical useful DIR compounds of this invention include:



Especially useful thio-substituted hydroquinones are the  $\alpha$ -(5-tetrazolylthio) hydroquinones and the  $\alpha$ -(2-benzoxazolyl) hydroquinones, such as compounds I through VI, below. The  $\alpha$ - in these names indicates that the substituent can be in any available position on the hydroquinone nucleus.

Ball is a ballast group as described above for DDR couplers.

Sol is an acidic solubilizing group as described above for DDR couplers.

Rad is a monothio radical which is split from the DIR compound when said compound cross-oxidizes with oxidized color developer. This —S— radical forms with "Rad" a diffusible mercaptan development inhibitor when the —S— is split from the DIR compound.

Rad includes a wide variety of photographically inert carbon containing heterocyclic radicals that are diffusible in the layers of the Color-Forming Unit and form mercaptans with the monothio connecting or linking radical when the connecting radical is split from the quinone of the DIR hydroquinone compound.

Typically such radicals generally contain at least one hetero nitrogen, oxygen or sulfur atom, and preferably, 1 to 4 hetero nitrogen atoms. The hetero nitrogen atoms in the heterocyclic radicals have no hydrogen atom attached thereto as the RAD radical is photographically inert. Illustrative carbon-containing heterocyclic radicals include 1-phenyl-tetrazolyls, oxazolyls, oxadiazolyls, diazolyls, thiadiazolyls, benzoxazolyls, benzothiazolyls, pyridinyls, pyridinyls, quinolinyls, and the like.

R=hydrogen, or any alkaline splittable masking group, such as an acyl group, e.g., acetyl, mono-, di- or trichloroacetyl, mono-, di- or trifluoroacetyl, perfluoroacetyl (e.g. butyryl), pyruvyl, alkoxaryl, nitrobenzoyl, cyano-benzoyl, etc.

R<sub>1</sub> as in R above.

Any combination of R and R<sub>1</sub> may be used.

The nature of the ballast groups (BALL) in the DIR compounds and DDR coupler compounds described above is not critical as long as they confer nondiffusibility to these compounds. Typical ballast groups exemplified hereinafter in the specific compounds disclosed include long chain alkyl radicals or several short chain alkyl radicals having e.g. 8-22 carbon atoms, linked directly or indirectly to the coupler molecules, as well as aromatic radicals of the benzene and naphthalene series, etc., linked directly or indirectly to the coupler molecules by a splittable linkage, or by a removable or irremovable but otherwise nonfunctional linkage depending upon the nature of the coupler compound. Useful ballast groups generally have at least 8 carbon atoms.

With regard to the above-described coupler radicals (COUP) in the DDR couplers, the "coupling position" is well known to those skilled in the photographic art. The 5-pyrazolone coupler radicals couple at the carbon atom in the 4-position, the phenolic coupler radicals, including  $\alpha$ -naphthols, couple at the carbon atoms in the 4-position and the open-chain ketomethylene coupler radicals couple at the carbon atom forming the methylene moiety, e.g.,



The term "nondiffusing" used herein as applied to the couplers and coupler reaction products, has the meaning commonly applied to the term in color photography and

denotes materials which for all practical purposes do not migrate or wander through organic colloid layers, such as gelatin, comprising the sensitive elements of the invention. The term "diffusible" as applied to the mercaptan development inhibitors released from the DIR compounds and the dyes released from the DDR couplers in the present processes has the converse meaning and denotes materials having the property of diffusing effectively through the colloid layers of the sensitive elements in the presence of the "nondiffusing" materials from which they are derived in alkaline color developing solutions.

The silver halide emulsion of the present photographic elements are conventional developing-out photographic silver halide emulsions including silver chloride, silver bromide, silver bromoiodide, silver chlorobromide and silver chlorobromoiodide emulsions. There can be employed as the dispersing agent or substrate for the silver halide in its preparation, gelatin or some other commonly employed photographic hydrophilic colloidal material such as colloidal albumin, a cellulose derivative, or a synthetic resin, for instance, a polyvinyl compound, although gelatin is preferred. Such hydrophilic colloidal materials can also be used in the non-light-sensitive layers in the subject elements in accordance with usual practice. Such hydrophilic colloids are well known in the art.

The subject photographic emulsions can contain the addenda generally utilized in such products including optical sensitizers, speed-increasing materials, antifoggants, coating aids, gelatin hardeners, plasticizers, ultraviolet absorbers and the like.

As described above, each Color-Forming Unit in the photographic elements of the invention contains, in addition to a light-sensitive silver halide emulsion (Component A), an emulsion of a water-insoluble metal salt that is developable (i.e., reducible to metal) with alkaline color developing solutions containing aromatic primary amino color developing agents to a substantial density without light exposure of the element (Component C). Such metal salts are preferably water-insoluble light-sensitive silver salts such as silver chloride, silver bromide, silver iodide, silver bromoiodide, silver chlorobromoiodide, silver citrate, silver oxalate, silver phosphate, silver stearate, silver, ferrocyanide, silver cyanide, silver thiocyanate and the like. Other useful salts include palladium

bromide, palladium cyanide and related heavy metal salts, as well as cuprous bromide and the like. Such metal salts can be made "spontaneously" developable by incorporating in the emulsion a wide variety of well-known physical development nuclei. Typical development nuclei include colloidal noble metals such as silver and gold; colloidal metal sulfides, selenides and tellurides such as lead sulfide, nickel sulfide, cadmium sulfide, silver sulfide, silver selenide, silver telluride, copper sulfide, zinc sulfide and mercury sulfide; metal proteinates such as silver proteinates; sodium sulfide; colloidal sulfur; and such organic sulfur compounds as thiourea, and xanthates. Conventional solvents for the metal salts are utilized in the developing compositions when the physical development nuclei are employed to make the emulsions "spontaneously" developable, including ammonium and alkali metal thiosulfates, thiocyanates, sulfites and the like. Another method that can be utilized to make the light-sensitive, water-insoluble salts "spontaneously" developable is by prefogging the emulsion with light or with chemical reducing agents such as alkali metal borohydrides and the like in accordance with well-known photographic fogging techniques.

A wide variety of alkaline color developing solutions containing aromatic primary amino color developing agents can be utilized to process the present photographic elements. Such developing solutions are utilized to develop or reduce to silver the exposed silver halide in the light-sensitive emulsions (Component A) to form a negative image, and to develop or reduce to a metal the metal salt in the "spontaneously" developable emulsion (Component C) to form a positive image. Particularly useful developing agents are the well-known p-phenylenediamine color developing agents. The color developing agent can be either incorporated in an alkaline photographic developing solution that is topically applied to the present photographic elements on processing, or the color developing agent can be incorporated in the element.

When the color developing agent is used in the present photographic elements, it is advantageous to use forms that have substantial stability in emulsions such as Schiff base derivatives of primary amino developing agents. Such Schiff bases are prepared by reacting primary amino developing agents with sulfonated, hydroxylated or carboxylated aromatic aldehydes of the benzene or naphthalene series. Such Schiff bases typically have the formula  $R-N=CH-R'$  wherein R is an aryl radical such as a phenyl radical substituted in the ortho or para position with a hydroxyl group or an amino group (e.g.  $-OH$ ,  $-NH_2$ ,  $-NHR'$  or  $-N(R'')_2$  wherein  $R''$  is a lower alkyl radical having 1 to 6 carbon atoms); and R' is an aryl radical such as phenyl or naphthyl substituted with an acidic group such as carboxyl, sulfo, and hydroxy lower alkyl groups. A typical Schiff base color developing agent can be prepared by reacting 2-amino-5-diethylaminotoluene and o-sulfonylbenzaldehyde. Other Schiff base developers that are useful as such, as salts or as sulfur dioxide complexes include:

- (1) N - ethyl - N - ( $\beta$  - hydroxyethyl) - 4 - (o-sulfonylbenzylideneamino)aniline sodium salt,
- (2) N - N - diethyl - 4(2,4 - dihydroxybenzylideneamino)-3-methylaniline, and
- (3) N - ethyl - 3 - methyl-N-( $\beta$ -methylsulfonamidoethyl)-4-(2-sulfonylbenzylideneamino)aniline sodium salt.

Such incorporated developing agents can be activated by immersing the photographic element in an aqueous alkaline solution or by spreading an aqueous alkaline solution on the surface of the element. Such incorporated developing agents can be positioned in any layer of the present photographic elements from which the developing agents can be readily made available for development on activation with aqueous alkaline solutions. Generally, such incorporated developing agents are either incorporated in the light-sensitive silver halide emulsion layers or in layers contiguous thereto.

Typical supports comprising the photographic elements of the invention include cellulose nitrate film, cellulose acetate film, polyvinyl acetal film, polystyrene film, polyethylene terephthalate film, polyethylene film, polypropylene film, and related films of resinous materials, as well as paper, glass, and others.

In preparing the photographic elements of the invention, the above-described emulsion layers are coated on the photographic supports in the form of multilayer color photographic elements having at least two preferably three Color-Forming Units sensitive to different regions of the visible spectrum. The uppermost Color-Forming Unit is preferably selectively sensitive to blue light. Between the blue light-sensitive Color-Forming Unit and the other Color-Forming Units there is typically disposed a yellow dye layer of Carey Lea silver layer for absorbing or filtering blue radiation that may be transmitted through the uppermost blue sensitive layer. However, the physical disposition of the red, green and blue light-sensitive Color-Forming Units within the present photographic elements can be widely varied in accordance with usual practice. Such multilayer photographic elements can also have other interlayers or sublayers for specialized purposes in accordance with usual practice.

Barrier layers are used between each Color-Forming Unit to ensure that the activity of the development inhibiting mercapto compounds released by the DIR compounds are confined to a single Color-Forming Unit. Hence, the barrier layers contain a water-insoluble salt or metal capable of forming a water-insoluble salt with mercaptans, silver halides such as silver chloride, silver bromide, silver iodide, silver bromoiodide, silver chlorobromoiodide, etc., being preferably used. Other compounds suitable for use in the present barrier layers that react with mercaptans include colloidal metals such as silver and gold; and colloidal metal sulfides, selenides and tellurides such as lead sulfide, nickel sulfide, cadmium sulfide, silver sulfide, copper sulfide, zinc sulfide, mercury sulfide, silver selenide, silver telluride and the like. The barrier layers containing light-sensitive silver salts are prepared to be substantially less sensitive to light than the light-sensitive emulsions in the Color-Forming Units. Such barrier layers also serve to prevent oxidized color developing agent from wandering from one Color-Forming Unit to another where it could cause color contamination. Antioxidants such as n-octadecyl hydroquinone and the like phenolic antioxidants, and nondiffusible photographic color couplers that form nondiffusible dyes on coupling with oxidized aromatic amino color developing agents can be utilized in the barrier layers to prevent wandering of such oxidized color developing agent.

The reception layer used to receive the diffused dye images on color development of the photoelements of the invention can be either a separate sheet pressed in contact with the photoelement or a layer integral with the photoelement.

When the reception layer is a separate reception sheet, the development and transfer operations can be effected by bathing either or both the exposed photographic element and the mordanted reception sheet in the developing solution before rolling into contact with each other. Alternatively, a viscous developing composition can be placed between the elements for spreading in a predetermined amount across and in contact with the exposed surface of the sensitive element so as to provide all of the solution required for the picture area. The viscous developing composition is desirably utilized in one or more pods integral with the photoelement or the reception sheet that can be readily ruptured when development is desired, suitable viscous developer utilization techniques being disclosed in U.S. Patents 2,543,181; 2,559,643; 2,647,049; 2,647,056; 2,661,293; 2,698,244; 2,698,798; and 2,774,668.

When the reception layer for receiving the diffusible dye is an integral part of the photosensitive assembly, it is also useful. A typical element of this type can com-

prise a support, a mordanted colloid layer thereon and the various emulsion layers described above coated thereover. When easily dissolved emulsions are used such as those containing polyvinyl alcohol or an alkali-soluble cellulose ether phthalate vehicles, or a wet or dry stripping layer containing such vehicles is provided between the emulsions and reception layer, the developed emulsion layers can then be readily separated from the reception layer leaving the dye image thereon. Similarly, the reception layer can be initially bonded to the outer emulsion surface. In this case, it is preferred to expose through the support of the sensitive element unless the reception layer itself is transparent. Such photoelements can be processed in the same manner as those not containing integral reception layers.

The reception layers in the photoelements of the invention can contain any of the conventional mordant materials for acid dyes. The reception layer can contain mordants such as polymers of amino guanidine derivatives of vinyl methyl ketone described in the Minsk U.S. Patent 2,882,156 granted Apr. 14, 1959. Other mordants include the 2-vinyl pyridine polymer metho-p-toluene sulfonate and similar compounds described in Sprague et al., U.S. Patent 2,484,430 granted Oct. 11, 1949 and cetyl trimethylammonium bromide, etc. Particularly effective mordanting compositions are described in copending applications of Whitmore, U.S. Ser. No. 211,095, filed July 19, 1962, now U.S. Patent 3,271,148, and Bush, U.S. Ser. No. 211,094 filed July 19, 1962, now U.S. Patent 3,271,147. The mordanting compositions described in the Knechel et al., application comprise at least one hydrophilic organic colloid containing a finely-divided, uniform dispersion of droplets or globules of a high-boiling, water-immiscible organic solvent in which is dissolved a high concentration of a cationic nonpolymeric, organic dye-mordanting compound for acid dyes. The mordanting compositions described in the Bush application comprise at least one hydrophilic organic colloid containing a finely-divided, uniform dispersion of particles of a salt of an organic acidic composition containing free acid moieties and a cationic, nonpolymeric, organic dye-mordanting compound for acid dyes. Useful cationic or basic organic dye-mordanting compounds for acid dyes include quaternary ammonium and phosphonium, and ternary sulfonium compounds in which there is linked to the N, P, or S onium atom at least one hydrophobic ballast group such as long-chain alkyl or substituted alkyl groups. Furthermore, the reception layer or sheet can be sufficient by itself to mordant the dye as in the case of the use of a sheet or layer of a polyamide or related polymeric material.

Reception sheets for the dye images, as well as the photoelements of the invention can contain ultraviolet absorbing materials. In the reception sheets, ultraviolet absorbers protect the mordanted dye images from fading and print-out due to ultraviolet light. In the photoelements, ultraviolet absorbers can serve as taking filters to reduce ultraviolet sensitivity. Typical ultraviolet absorbing materials are described in copending applications of Sawdey, U.S. Ser. Nos. 144,228 filed Oct. 10, 1961, now U.S. Patent 3,253,921 and 183,417 filed Mar. 29, 1962, now U.S. Patent 3,250,617. Illustrative useful ultraviolet absorbing materials disclosed by Sawdey have the formulas



and



wherein: R is a phenyl group including such substituents as hydrogen atoms, halogen atoms, alkyl groups, alkoxy groups or hydroxy groups; and R<sub>1</sub>, R<sub>2</sub> and R<sub>3</sub> are hydrogen atoms, hydroxyl groups, halogen atoms, nitro groups, alkyl groups, alkoxy groups, aryl groups or aryloxy groups. Other ultraviolet absorbing materials well known in the photographic art can also be utilized.

If desired, a "keep-negative" as well as a positive color transfer print can be prepared. In preparing such a color negative, a conventional photographic color coupler of the type that forms a nondiffusible dye when reacted with oxidized color coupler is utilized with the DIR compound. In this embodiment, DDR couplers are chosen that do not form colored nondiffusible dyes during the present process. Also, the reception layer used to receive the diffused positive dye image is a separate receiving sheet not integral with the element. After the positive image is transferred to the receiving sheet, the remaining negative element is fixed in hypo to remove unexposed silver halide and bleached (i.e., with an alkali metal ferricyanide) to remove silver. Suitable photographic color couplers that form nondiffusible dyes are of the phenolic, 5-pyrazolone and open-chain ketomethylene type such as those disclosed in Spence et al., U.S. Patent 2,640,706; Weissberger et al., U.S. Patent 2,407,210; and Weissberger et al., U.S. Patent 2,474,293.

The drawings illustrate in section and in elevation typical photographic elements of the invention.

FIG. 1 illustrates a typical photographic element of the invention wherein the DIR compound is positioned in the light-sensitive silver halide emulsion and the "spontaneously" developable emulsion comprises a nucleated metal salt in each Color-Forming Unit.

FIG. 2 illustrates a typical photographic element of the invention wherein the DIR compound is positioned in the light-sensitive silver halide emulsion and the "spontaneously" developable emulsion comprises a fogged silver halide emulsion in each Color-Forming Unit.

In FIG. 1, over photographic support 10 are coated three Color-Forming Units of the invention that are sensitive to different regions of the spectrum. Over support 10 is coated nucleated metal salt layer 11 containing a cyan-forming DDR coupler. Over layer 11 is coated a silver halide emulsion that is sensitive to red light and a DIR compound. Over layer 12 is coated barrier layer 13 containing a compound capable of forming an insoluble salt with mercaptans. Over layer 13 is coated nucleated metal salt layer 14 containing a magenta-forming DDR coupler. Over layer 14 is coated silver halide emulsion layer 15 that is sensitive to green light and a DIR compound. Over layer 15 is coated barrier layer 16 containing a compound capable of forming an insoluble salt with mercaptans and a yellow filter material. Over layer 16 is coated nucleated metal salt layer 17 containing a yellow-forming DDR coupler. Over layer 17 is coated a silver halide emulsion layer 18 that is sensitive to blue light and a DIR compound.

With respect to FIG. 2, on photographic support 20 are coated three Color-Forming Units of the invention that are sensitive to different regions of the visible spectrum. On support 20 is coated fogged silver halide emulsion layer 21 containing a magenta-forming DDR coupler. Over layer 21 is coated silver halide emulsion layer 22 that is sensitive to green light and contains a DIR compound. Over layer 22 is coated barrier layer 23 containing a compound capable of forming an insoluble salt with mercaptans. Over layer 23 is coated fogged silver halide emulsion layer 24 containing a cyan-forming DDR coupler. Over layer 24 is coated silver halide emulsion layer 25 that is sensitive to red light and contains a DIR compound. Next, barrier layer 26 containing a compound capable of forming an insoluble salt with mercaptans and a yellow filter material is coated. Over layer 26 is coated fogged silver halide emulsion layer 27 containing a yellow-forming DDR

coupler. Over layer 27 is coated silver halide emulsion layer 28 that is sensitive to blue light and contains a DIR compound. Over layer 28 is coated protective layer 29.

2-[4-[3-(4-tert-amyl - x - sulfophenoxy)benzamido]phenethyl]-x-(1-phenyl-5 - tetrazolylthio)hydroquinone diacetate sodium salt dihydrate



The development inhibitor releasing compounds (DIR) compounds) used in my invention are described by the following specific examples:

2{4-[3-(4-tert-amyl - x - sulfophenoxy)benzamido]phenethyl}-x-(1-phenyl-5-tetrazolylthio)hydroquinone sodium salt

20



5-[4-(3,5 - disulfobenzamido)phenethyl] - 2-methyl-3-(1-phenyl-5-tetrazolylthio)hydroquinone disodium salt

35

2-[4-(3,5-disulfobenzamido)phenethyl] - x - (1-phenyl-5-tetrazolylthio)-hydroquinone disodium salt dihydrate



2-{4-[2-(2,4-di-tert-amylphenoxy) - 5 - (3,5-disulfobenzamido)phenethyl] - x - (1-phenyl-5-tetrazolylthio)hydroquinone disodium salt dihydrate

45



65 2-[4-(3,5-disulfobenzamido)phenethyl]-x-(2-benzoxazolylthio)hydroquinone disodium salt dihydrate



The following synthesis illustrates the preparation of a representative DIR hydroquinone compound of my invention.

*Compound I.*—2-{4-[3-(4-t-amyl-x-sulfophenoxy)benzamido]phenethyl}-x-(1-phenyl-5-tetrazolylthio)hydroquinone sodium salt

A solution of 8 parts of Intermediate #5 below in 100 volumes of methyl alcohol was refluxed under nitrogen for 3 hours. To the clear amber solution was then added a solution of 1 part  $\text{NaHCO}_3$  in 20 volumes of  $\text{H}_2\text{O}$ . This clear reaction mixture was concentrated to dryness in vacuo to yield 7 parts of tan powder.

*Intermediate #1.*—4-trifluoroacetamidophenethylhydroquinone

143 parts of 4-aminophenethylhydroquinone were added to 600 volumes of trifluoroacetic anhydride. The clear mixture was refluxed for 5 minutes on a water bath and poured slowly into 3000 volumes of water whereupon the product separated in the form of a tan solid which was filtered off and dried.

*Intermediate #2.*—4-trifluoroacetamidophenethylbenzoquinone

40 parts of Intermediate #1 was dissolved in 1000 volumes of acetone and 60 volumes of  $\text{H}_2\text{O}$ . To this solution was added dropwise at  $-10^\circ$  a solution of 60 volumes of concentrated  $\text{H}_2\text{SO}_4$  in 100 volumes of  $\text{H}_2\text{O}$  over a period of 20 minutes. To this solution was added dropwise at  $-5^\circ$  over a period of 20 minutes a solution of 18 parts of potassium dichromate in 100 volumes of  $\text{H}_2\text{O}$ . This mixture was stirred for 5 minutes after which time 2000 volumes of water were added whereupon the product separated. This mixture was stirred for 1 hour and the solid product was filtered off and dried.

*Intermediate #3.*—X-(1-phenyl-5-tetrazolylthio)-2-(4-trifluoroacetamidophenethyl)hydroquinone

To a solution of 48.5 parts of Intermediate #2 in 500 volumes of chloroform under nitrogen was added with stirring 27 parts of 1-phenyl-5-mercaptopetrazole. This mixture was refluxed under nitrogen for 3 hours during which time solution occurred and the product separated in the form of a white solid. This solid was filtered off and dried.

*Intermediate #4.*—2-(4-aminophenethyl)-x-(1-phenyl-5-tetrazolylthio)hydroquinone

To a solution of 25 parts of Intermediate #3 in 500 volumes of 90 percent ethyl alcohol under nitrogen was added 25 volumes of 20 percent  $\text{NaOH}$ . The clear reaction mixture was let stand overnight at room temperature under nitrogen, after which time it was poured into 2000 volumes of dilute acetic acid. The tan solid, which separated, was filtered off and dried.

*Intermediate #5.*—2-{4-[3-(4-t-amyl-x-chlorosulfonylphenoxy)benzamido]phenethyl}-x-(1-phenyl-5-tetrazolylthio)hydroquinone

To a solution of 16 parts of Intermediate #4 and 5 parts of  $\text{N,N}$ -dimethylaniline in 500 volumes of dry acetone was added at  $40^\circ$  with stirring, a solution of 16 parts of 3-(4-t-amyl-x-chlorosulfonylphenoxy)benzoyl chloride in 50 volumes of dry acetone. The clear reaction mixture was refluxed for 4 hours and then poured into 500 volumes of  $\text{H}_2\text{O}$ . The gummy solid was dissolved in 500 volumes of benzene and poured into 500 volumes of cyclohexane. The white solid which separated was filtered off and dried.

The following are representative DDR couples of the invention, to wit, nondiffusible coupler compounds that release or form diffusible acid dyes on coupling with the oxidation products of color developing agents.

Couplers VII to XVI below are substituted in the coupling position with preformed yellow dyes that are split from the ballasted couplers and become diffusible when said couplers react with oxidized color developers.

1-hydroxy-4-{3-[4-(N-ethyl-N- $\beta$ -sulfoethylamino)-2-methylphenylazo]phenylazo}-N-[ $\delta$ -(2,4-di-tert-amylphenoxy)butyl]-2-naphthamide sodium salt.



20

30

1-hydroxy-4-{4-[1-(4-sulfophenyl)-3-methyl-4-pyrazol-5-onylazo]-3-sulfophenylazo}-N-[ $\delta$ -(2,4-di-tert-amylphenoxy)butyl]-2-naphthamide disodium salt.



40

55

1-hydroxy-4-{3-[4-(N-ethyl-N- $\beta$ -carboxyethylamino)-2-methylphenylazo]phenylazo}-N-[ $\delta$ -(2,4-di-tert-amylphenoxy)butyl]-2-naphthamide sodium salt.



15

1-hydroxy-4-(2,4-dinitrophenylthio)-N-[ $\delta$ -(2,4-di-tert-  
amylphenoxy)butyl]-2-naphthamide



16

1 - hydroxy - 4 - {4-[3-methyl-4-(1,5-disulfo-3-naphthyl-  
azo) - 1 - pyrazol - 5-onyl]phenylazo}-N-[ $\delta$ -(3-penta-  
decylphenoxy)butyl]-2-naphthamide disodium salt

5 XIII.

10

15

20



1-hydroxy-4-{4-[1-(4-sulfophenyl)-3-methyl-4-pyrazol-  
5-onylazo]-3-sulfophenylazo}-N-4-[ $\alpha$ -(2,4-di-tert-amyl-  
phenoxy)butyramido]phenethyl}-2-naphthamide di-  
potassium salt. 25

XI.



1-hydroxy-4-{4-[3-methyl-4-(1,5-disulfo-3-naphthylazo)-  
1-pyrazol-5-onyl]phenylazo}-N-{4-[ $\alpha$ -(2,4-di-tert-  
amylphenoxy)butyramido]phenethyl}-2-naphthamide  
dipotassium salt.

55

XII.



1 - (p - t - butylphenoxyphenyl)-3-[ $\alpha$ -(4-t-butylphenoxy) propionamido] - 4 - (2 - bromo-4-methylamino-5-sulfo-1-anthra-9,10-quinonylazo)-5-pyrazolone

Each of the Couplers XVII to LII below contain an acid solubilizing group in a noncoupling position and on coupling with oxidized color developer forms a nondiffus-

XIV.



$\alpha$  - {3 - [ $\alpha$ -(2,4-di-tert-amylphenoxy)acetamido]benzoyl}-  
 $\alpha$  - {3 - [4-(N-ethyl-N- $\beta$ -sulfoethylamino)-2-methylphenylazo]phenylazo} - 2-methoxyacetanilide sodium salt

25 ible dye by the elimination of a ballasting group from the coupling position as a direct result of said coupling reaction.

XV.



1 - hydroxy - 4-{4-[1-(4-sulfophenyl)-3-carboxy-4-pyrazol - 5 - onylazo]-3-sulfophenylazo}-N-{4-[ $\alpha$ -(2,4-di-tert - amylphenoxy)butyramido]phenyethyl} - 2 - naphthamide

Couplers XVII to XXXV below form diffusible cyan 45 dyes.

XVI.



19

1-hydroxy-4-stearoyloxymercuri-2-naphthoic acid  
XVII.



1-hydroxy-4-dodecyloxy-2-naphthoic acid  
XVIII.



1 - hydroxy - 4-(4-octadecyloxyphenylazo)-2-naphthoic acid  
XIX.



1 - hydroxy - 4 - (4-octadecyloxyphenylazo) - N-[ $\beta$ -(3,5-disulfobenzamido)ethyl] - 2 - naphthamide dipotassium salt  
XX.



1 - hydroxy - N - (<math>\beta</math>-sulfoethyl)-4-(4-octadecyloxyphenylazo)-2-naphthamide potassium salt  
XXI.



20

1 - hydroxy - 4 - (4-octadecyloxyphenylazo)-3'-carboxy-4'-hydroxy-2-naphthanilide

XXII.



15

20 1 - hydroxy - 3',5'-dicarbomethoxy-4-dodecyloxy-2-naphthanilide

XXIII.



25

30 1 - hydroxy - 4 - (2-hydroxy-4-pentadecylphenylazo)-N-ethyl-3',5'-dicarboxy-2-naphthanilide

XXIV.



40

45

50

1-hydroxy-4-octadecyloxy-N-ethyl-3',5'-dicarboxy-2-naphthanilide

XXV.



55

60

65 1-hydroxy-4-(3-octadecylcarbamylphenylthio)-N-ethyl-3',5'-dicarboxy-2-naphthanilide

XXVI.



70

75

21

4,4'-p-octadecyloxybenzylidenebis(1-hydroxy-N-ethyl-3',5'-dicarboxy-2-naphthanilide)

XXVII.

5  
10

1-hydroxy-5-acetamido-4-octadecyloxy-8-phenylazo-2-naphthoic acid

XXVIII.

15  
20  
25

2-(3,5-disulfobenzamido)-5-methyl-4-(4-octadecyloxyphenylazo) phenol dipotassium salt

XXIX.

35  
40  
45

2-(3,5-disulfobenzamido)-4-(4-hydroxy-2-pentadecylphenylazo)-5-methylphenol dipotassium salt

XXX.

50  
55  
60

2-(3,5-dichlorosulfonylbenzamido)-5-methyl-4-(4-nitrophenylthio)phenol

XXXI.



(Hydrolyze to acid while dispersing) 75

65 Couplers XXXVI to XLVII below form diffusible magenta dyes.

1-phenyl-3-(3-sulfobenzamido)-4-(4-octadecyloxyphenylazo)-5-pyrazolone sodium salt

70 XXXVI.



23

1-phenyl-3-(3,5-disulfobenzamido)-4-(4-octadecyloxy-phenylazo)-5-pyrazolone disodium salt

XXXVII.



1 - [4 - (4 - t - butylphenoxy)phenyl] - 3 - (3,5 - di-sulfobenzamido)-4-(4-octadecyloxyphenylazo)-5-pyrazolone dipotassium salt

XXXVIII.



1-phenyl-3-(3,5-disulfobenzamido)-4-(4-hydroxy-2-pentadecylphenylazo)-5-pyrazolone dipotassium salt

XXXIX.



1-(p-sulfophenyl)-3-carboxymethyl-4-(4-hydroxy-2-pentadecylphenylazo)-5-pyrazolone sodium salt

XL.



1-(4-sulfophenyl)-3-carboxy-4-(4-hydroxy-2-pentadecylphenylazo)-5-pyrazolone sodium salt

XLI.



1 - phenyl - 3 - (3,5 - disulfobenzamido) - 4 - [4 - (3-methyl - 5 - pentadecyl)pyrazolylazo] - 5 - pyrazolone dipotassium salt

XLII.



1-(4-sulfophenyl)-3-(4-sulfoanilino)-4-(2-hydroxy-4-pentadecylphenylazo)-5-pyrazolone dipotassium salt

XLIII.



23

24

1-(4-sulfophenyl)-3-(4-sulfoanilino)-4-(2-amino-4-pentadecylphenylazo)-5-pyrazolone dipotassium salt

XLIV.



5

10

15

20

25

30

35

40

45

50

55

60

65

70

75

1-[4-(3,5-dicarboxybenzamido)phenyl]-3-ethoxy-4-(3-octadecylcarbamylphenylthio)-5-pyrazolone

XLV.



1-(4-sulfophenyl)-3-(4-sulfoanilino)-4-(3-octadecylcarbamylphenylthio)-5-pyrazolone disodium salt

XLVI.



4,4'-(4-octadecyloxybenzylidene)bis[1-phenyl-3-(3,5-disulfobenzamido)-5-pyrazolone]tetra potassium salt

XLVII.



60

65

70

75

25

Couplers XLVIII to LII below form diffusible yellow dyes.

$\alpha$ -Benzoyl- $\alpha$ -(4-hydroxy-2-pentadecylphenylazo)-4-(3-sulfobenzamido)acetanilide sodium salt

XLVIII.



$\alpha$ -Benzoyl- $\alpha$ -(4-hydroxy-2-pentadecylphenylazo)-4-(3,5-disulfobenzamido)acetanilide dipotassium salt

XLIX.



$\alpha$ -Benzoyl- $\alpha$ -(4-[3-methyl-5-pentadecyl]pyrazolylazo)-4-(3,5-disulfobenzamido)acetanilide dipotassium salt

L.



$\alpha$ -Benzoyl- $\alpha$ -(3-octadecylcarbamylphenylthio)-3,5-dicarboxyacetanilide

LI.



$\alpha$ -Pivalyl- $\alpha$ -(3-octadecylcarbamylphenylthio)-4-sulfoacetanilide potassium salt

LII.



Diffusible dyes are formed when the above listed (i.e. VII to LII) non-diffusing couplers are employed in the process of the invention with well-known p-phenylenediamine developing agents, e.g., N,N-diethyl-p-phenylenediamine, 2-amino-5-diethylamino toluene, N-ethyl- $\beta$ -methanesulfonamidoethyl-3-methyl-4-aminoaniline, and other

70

75

26

N,N-dialkyl-p-phenylenediamine developing agents described by Bent et al. J.A.C.S. 73, 3100-3125 (1951).

Couplers LIII to LXI are nondiffusible couplers which can also be used in the process of my invention when the color developing agent is supplied with the alkali solubilizing function.

Couplers LIII to LVI below form diffusible cyan dyes. 1-hydroxy-4-(4-octadecyloxyphenylazo)-N-methyl-2-naphthanilide

10 LIII.

15



LIV.

20



LV.

25

30

35

40

45

50

55

60

65

70

75

80

85

90

95

100

105

110

115

120

125

130

135

140

145

150

155

160

165

170

175

180

185

190

195

200

205

210

215

220

225

230

235

240

245

250

255

260

265

270

275

280

285

290

295

300

305

310

315

320

325

330

335

340

345

350

355

360

365

370

375

380

385

390

395

400

405

410

415

420

425

430

435

440

445

450

455

460

465

470

475

480

485

490

495

500

505

510

515

520

525

530

535

540

545

550

555

560

565

570

575

580

585

590

595

600

605

610

615

620

625

630

635

640

645

650

655

660

665

670

675

680

685

690

695

700

705

710

715

720

725

730

735

740

745

750

755

760

765

770

775

780

785

790

795

800

805

810

815

820

825

830

835

840

845

850

855

860

865

870

875

880

885

890

895

900

905

910

915

920

925

930

935

940

945

950

955

960

965

970

975

980

985

990

995

995

1000



1-hydroxy-4-(4-octadecyloxyphenylazo)-N-methyl-2-naphthanilide



1-hydroxy-4-(2-amino-4-octadecyloxyphenylazoxy)-2-naphthamide



1-hydroxy-2',5'-dibutoxy-4-[4-(sulfomethyl)phenylazo]-2-naphthanilide

Couplers LVII to LIX below form diffusible magenta dyes.

1-phenyl-3-methyl-4-(4-octadecyloxybenzylidene)-5-pyrazolone

LVII.



4,4'-thiobis(1-phenyl-3-methyl-5-pyrazolone)

LVIII.



4,4'-dithiobis(1-phenyl-3-methyl-5-pyrazolone)

LIX.



Couplers LX and LXI below form diffusible yellow dyes.

$\alpha, \alpha'$ -(4-octadecyloxybenzylidene)bis[ $\alpha$ -benzoylacetanilide]

LX.



$\alpha, \alpha'$ -Dithiobis[benzoylacetanilide]

LXI.



Representative color developing agents possessing the solubilizing functions useful with the nondiffusing couplers above are as follows:

4-amino-N-ethyl-3-methyl-N-( $\beta$ -sulfoethyl)aniline  
4-amino-N-ethyl-3-methoxy-N-( $\beta$ -sulfoethyl)aniline  
4-amino-N-ethyl-N-( $\beta$ -hydroxyethyl)aniline  
4-amino-N,N-diethyl-3-hydroxymethylaniline  
4-amino-N-methyl-N-( $\beta$ -carboxyethyl)aniline  
4-amino-N,N-bis( $\beta$ -hydroxyethyl)aniline  
4-amino-N,N-bis( $\beta$ -hydroxyethyl)-3-methylaniline  
3-acetamido-4-amino-N,N-bis( $\beta$ -hydroxyethyl)aniline  
4-amino-N-ethyl-N-(2,3-dihydroxypropyl)-3-methyl-aniline sulfate salt  
4-amino-N,N-diethyl-3-(3-hydroxypropoxy)aniline

When the DDR couplers given above were incorporated into exposed silver halide emulsions that were developed in contact with a mordanted reception layer using an alka-

line color developing composition containing the developing agent 4-amino-N-ethyl-N-( $\beta$ -hydroxyethyl)aniline, the following colors of dye images were obtained on the reception layer from the respective couplers:

|    |         |               |
|----|---------|---------------|
| 5  | VII     | yellow        |
|    | VIII    | yellow        |
|    | IX      | yellow        |
|    | X       | orange-yellow |
|    | XI      | yellow        |
| 10 | XII     | yellow        |
|    | XIII    | yellow        |
|    | XIV     | yellow        |
|    | XV      | yellow        |
|    | XVI     | yellow        |
| 15 | XVII    | cyan          |
|    | XVIII   | cyan          |
|    | XIX     | cyan          |
|    | XX      | cyan          |
| 20 | XXI     | cyan          |
|    | XXII    | cyan          |
|    | XXIII   | cyan          |
|    | XXIV    | cyan          |
|    | XXV     | cyan          |
|    | XXVI    | cyan          |
| 25 | XXVII   | cyan          |
|    | XXVIII  | cyan          |
|    | XXIX    | cyan          |
|    | XXX     | cyan          |
| 30 | XXXI    | cyan          |
|    | XXXII   | cyan          |
|    | XXXIII  | cyan          |
|    | XXXIV   | cyan          |
|    | XXXV    | cyan          |
| 35 | XXXVI   | magenta       |
|    | XXXVII  | magenta       |
|    | XXXVIII | magenta       |
|    | XXXIX   | magenta       |
|    | XL      | magenta       |
| 40 | XLI     | magenta       |
|    | XLII    | magenta       |
|    | XLIII   | magenta       |
|    | XLIV    | magenta       |
|    | XLV     | magenta       |
| 45 | LXVI    | magenta       |
|    | XLVII   | magenta       |
|    | XLVIII  | yellow        |
|    | XLIX    | yellow        |
| L  | L       | yellow        |
| 50 | LI      | yellow        |
|    | LII     | yellow        |

The following syntheses illustrate the methods for preparations of representative DDR couplers of my invention.

*Coupler VII.* — 1-hydroxy-4-{3-[4-(N-ethyl-N- $\beta$ -sulfoethylamino)-2-methylphenylazo]phenylazo}-N-[ $\delta$ -(2,4-di-tert-amylphenoxy)butyl]-2-naphthamide sodium salt

To 200 ml. of concentrated sulfuric acid at 10° C. was added with stirring 17 grams of Intermediate C below. To the resultant solution was added dropwise over a period of 30 minutes at -5° C. with stirring a solution of 3.5 grams of sodium nitrite in 35 ml. of concentrated sulfuric acid (i.e. nitrosylsulfuric acid solution). This solution was stirred for a total of two hours after which time it was poured on to crushed ice. This solution was then added to a solution of 21 grams of 1-hydroxy-N-[ $\delta$ -(2,4-di-tert-amylphenoxy)butyl]-2-naphthamide (U.S. Patent 2,474,293), in two liters of pyridine over a 30-minute period with stirring at 0-5° C. After 12 hours at room temperature the reaction mixture was mixed with 1.5 kg. of crushed ice and acidified with concentrated hydrochloric acid. The red solid which separated was collected, washed with water and recrystallized twice from glacial acetic acid, yielding the product.

*Coupler VII: Intermediate A.—N-ethyl-3-methyl-N-( $\beta$ -sulfoethyl)aniline sodium salt*

A mixture of 675 grams of N-ethyl-toluidine and 528 grams of sodium 2-bromoethane sulfonate was heated at 160–190° C. for 3½ hours, after which time mixture was cooled and 1200 ml. of water was added. The solution was made alkaline with sodium hydroxide and the solid which separated was collected, washed with acetone and ether and recrystallized from 2.5 liters of ethyl alcohol, yielding 420 grams of product.

*Coupler VII: Intermediate B.— $\beta$ -{N-ethyl-N-[3-methyl-4-(3-nitrophenylazo)phenyl]amino}-ethylsulfonic acid sodium salt*

To a solution of 27 grams of Intermediate A above in 250 ml. of water at 0° C. was added a chilled diazonium solution consisting of 14 grams of m-nitroaniline and 7.5 grams of sodium nitrite in 200 ml. of 6 N-hydrochloric acid. The resultant mixture was neutralized to Congo Red paper by the addition of sodium acetate. This mixture was chilled for 2 hours after which time the solid which separated was collected, washed with cold water, and recrystallized from 360 ml. of water, yielding a green product.

*Coupler VII: Intermediate C.— $\beta$ -{N-[4-(3-aminophenylazo)-3-methylphenyl]-N-ethylamino}ethyl sulfonic acid sodium salt*

To a solution of 41 grams of Intermediate B above in 2 liters of water at 90° C. was added over a period of 30 minutes a solution of 40 grams of 60 percent sodium sulfide in 150 ml. of water. The mixture was refluxed for an additional 2½ hours during which time approximately ½ of the water was distilled off. This mixture was filtered and refrigerated over night during which time a solid separated. The solid was collected and recrystallized from 200 ml. of ethyl alcohol, yielding the product.

*Coupler XIII: 1-hydroxy-4-{4-[3-methyl-4-(1,5-disulfo-3-naphthylazo)-1-pyrazol-5-onyl]phenylazo} - N - [ $\delta$ (3-pentadecylphenoxy)butyl] - 2 - naphthamide disodium salt*

A solution of 6.5 grams of sodium nitrite in 93 ml. of water was added to a solution of 49.5 grams of Intermediate E below in 300 ml. of five percent sodium carbonate solution. This mixture was cooled to 10° C. and added to a well-stirred mixture of 75 ml. concentrated hydrochloric acid and 150 grams of ice. After 1½ hours, the diazonium suspension was added in portions with vigorous stirring to a solution of 44.4 grams of Intermediate C below in a mixture of 1500 ml. of ethyl alcohol and 55 grams of potassium carbonate in 360 ml. water. After two hours, the crude product was filtered, triturated in boiling ethyl alcohol, then dissolved in 1500 ml. ethyl alcohol and 1500 ml. of 3 percent potassium carbonate solution. The dark orange solution was filtered and acidified with acetic acid. The solid which separated was filtered, triturated in acetone and benzene, extracted twice with hot water, and recrystallized from a 1:1 n-propyl alcohol-water mixture, yielding 40 grams of product, M.P.>270° C.

*Coupler XIII: Intermediate A.— $\gamma$ (3-pentadecylphenoxy)butyronitrile*

A mixture of 4 grams of sodium hydroxide and 31 grams of 3-pentadecylphenol (Minn. Mining and Mfg. Co.) in 100 ml. of xylene was refluxed for 6 hours during which time 1.8 ml. of water was distilled off. To the mixture was added 11 grams of  $\gamma$ -chlorobutyronitrile dropwise over 1 hour after which time the mixture was refluxed for 7 hours. The xylene was then distilled off over a 12 hour period and the residual oil was poured into 25 ml. of dilute hydrochloric acid. The waxy solid which separated was collected and recrystallized from 100 ml.

of acetonitrile, yielding 23 grams of product, M.P. 46–47° C.

*Coupler XIII: Intermediate B.— $\delta$ (3-pentadecylphenoxy)butylamine*

5 A mixture of 5 grams of Intermediate A above, 3 ml. of ethyl alcohol, 5 ml. of liquid anhydrous ammonia and 0.1 gram of Raney nickel was heated for 12 hours at 100° C. under a hydrogen atmosphere at a pressure of 2200 10 p.s.i. The cooled solution was filtered and concentrated in vacuo. The residual oil was distilled at 165° C. at 9 microns, yielding the product.

*Coupler XIII: Intermediate C.—1-hydroxy-N-[ $\delta$ (3-pentadecylphenoxy)butyl]-2-naphthamide*

A mixture of 5 grams of phenyl 1-hydroxy-2-naphthoate and 7 grams of Intermediate B above was heated at 150° C. for ½ hour in vacuo during which time phenol was collected from the mixture. The residual oil 20 was poured into 100 ml. of petroleum ether whereupon a crystalline solid separated. This solid was collected and recrystallized from 90 ml. of ethyl alcohol, yielding 8 grams of product, M.P. 64–66° C.

*Coupler XIII: Intermediate D.—1 - (4 - nitrophenyl)-3-methyl-4-(1,5-disulfo-3-naphthylazo)-5-pyrazolone di-sodium salt*

To a solution of 2.8 grams of 1-(4-nitrophenyl)-3-30 methyl-5-pyrazolone, 0.5 grams of sodium hydroxide and 7 grams of sodium acetate in 40 ml. of water was added 20° C. over a period of 20 minutes a diazonium mixture consisting of 1.1 gram of 2-amino-1,5-naphthalenedisulfonic acid disodium salt, 1.4 gram of sodium nitrite, 2 ml. of concentrated sulfuric acid and 10 ml. of water. The mixture was stirred for 1 hour at room temperature and heated over steam until all solids dissolved. The solution was cooled to 5° C. whereupon a red solid separated and was collected, yielding 4.5 grams of product.

*Coupler XIII: Intermediate E.—1 - (4-aminophenyl)-3-methyl - 4 - (1,5-disulfo-3-naphthylazo)-5-pyrazolone di-sodium salt*

To a mixture of 31 grams of Intermediate D above in 45 32 ml. of water at 90° C. was added over a period of 20 minutes a solution of 18 grams of 60 percent sodium sulfide in 40 ml. of water. The mixture was heated at reflux for an additional 2 hours after which time it was cooled to 50° C. and acidified with acetic acid. The solid which 50 separated was collected and recrystallized from 250 ml. of 10 percent brine solution, yielding 15 grams of product, M.P.>250° C.

*Coupler XVII: 1-hydroxy-4-stearoyloxymercuri-2-naphthoic acid*

To a solution of 9.4 grams of 1-hydroxy-2-naphthoic acid (J.A.C.S. 64, 799 (1942)) in 200 ml. of dioxane was added a solution of 38 grams of mercuric stearate in 500 ml. of dioxane. The mixture was heated over steam for 60 5 hours during which time a white solid separated. This solid was collected, washed with hot methyl alcohol and dried, yielding 30 grams of product.

*Coupler XVIII: 1-hydroxy-4-dodecyloxy-2-naphthoic acid*

To a suspension of 2 grams of 1,4-dihydroxy-2-naphthoic acid (J.A.C.S. 64, 799 (1942)) in 40 grams of lauryl alcohol was added dry hydrogen chloride gas at 90° C. 70 over a period of 11 hours while stirring. The clear reaction mixture was left at room temperature over night during which time a white solid separated. This solid was filtered, slurried in 50 volumes of petroleum ether, re-filtered and dried, yielding 1.25 grams of product, M.P. 135–136° C.

*Coupler XXI: 1-hydroxy-N-(β-sulfoethyl)-4-(4-octadecyloxyphenylazo)-2-naphthamide potassium salt*

To a solution of 51 grams of potassium hydroxide and 63 grams of Intermediate A below in 350 ml. of water and 1700 ml. of ethyl alcohol was added at 5° C. over a period of 1 hour, a diazonium solution consisting of 72 grams of Intermediate B below, 120 grams of p-toluene sulfonic acid, and 30 grams of isoamyl nitrite in 2 liters of n-propyl alcohol. The mixture was stirred at room temperature for 5 hours after which time 3 liters of water were added and the mixture brought to reflux. The hot solution was filtered, acidified with glacial acetic acid and cooled whereupon a solid separated. The solid was collected, recrystallized from 1.5 liters of n-butyl alcohol, yielding 80 grams of product, M.P. 228-30° C.

*Coupler XXI: Intermediate A.—1-hydroxy-N-(β-sulfoethyl)-2-naphthamide potassium salt*

A mixture of 132 grams of phenyl 1-hydroxy-2-naphthoate, 1 liter of ethyl alcohol, 57.5 grams of taurine, 300 ml. of water and 28 grams of potassium hydroxide was refluxed for 15 hours after which time the solution was cooled and the solid which separated was collected, washed with ethyl alcohol, recrystallized from H<sub>2</sub>O and dried, yielding 71 grams of product, M.P. 284-286° C.

*Coupler XXI: Intermediate B.—4-octadecyloxyaniline*

A mixture of 39 grams of 4-nitrophenyloctadecyl ether (J.A.C.S. 73, 458 (1951)) and 0.5 gram of 10 percent palladium on charcoal in 300 ml. of ethyl alcohol was heated at 50° C. for 1/2 hour under a hydrogen atmosphere at a pressure of 50 p.s.i.

The catalyst was filtered from the hot solution which was then chilled whereupon a solid separated. This solid was collected, and dried, yielding 32 grams of product, M.P. 78-81° C.

The preparations for couplers XXIV, XXV, XXVI and XXVII are given in copending application U.S. Ser. No. 154,841, filed Nov. 24, 2961, now abandoned.

*Coupler XXX: 2-(3,5-disulfonylbenzamido)-4-(4-hydroxy-2-pentadecylphenylazo) - 5-methylphenol dipotassium salt*

To a solution of 21 grams of 2-(3,5-dichlorosulfonylbenzamido)-5-methylphenol in 50 ml. of pyridine and 10 ml. of water was added a diazonium solution consisting of 16 grams of 4-amino-3-pentadecylphenol, 7 grams of isoamyl nitrite, and 10 ml. of concentrated hydrochloric acid in 100 ml. of n-propyl alcohol. The mixture was stirred at room temperature for 12 hours after which time it was poured into 400 ml. of saturated potassium chloride solution. The gummy solid which separated was collected, triturated twice in methyl alcohol and dried, yielding 11 grams of product.

*Coupler XXXVI: 1-phenyl-3-(3-sulfonylbenzamido)-4-(4-octadecyloxyphenylazo)-5-pyrazolone sodium salt*

To a solution of 3.6 grams of Intermediate B below and 2 grams of sodium hydroxide in 55 ml. of 90 percent ethyl alcohol at 0° C. was added with stirring a diazonium solution consisting of 3.6 grams of 4-octadecyloxyaniline (Intermediate B of Coupler XXI above), 5.7 grams of p-toluenesulfonic acid monohydrate and 1.5 grams of isoamyl nitrite in 100 ml. of n-propyl alcohol at 20° C. The mixture was stirred at room temperature for 3 hours after which time 25 ml. of water was added and the mixture was acidified with acetic acid. To this solution at 90° C. was added 100 grams of sodium chloride and the resultant solution was filtered and cooled. The solid which separated was collected, washed with water and dried, yielding 6 grams of product, M.P. 198-200° C.

*Coupler XXXVI: Intermediate A.—1-phenyl-3-(3-chlorosulfonylbenzamido)-5-pyrazolone*

To a solution of 88 grams of 1-phenyl-3-amino-5-pyrazolone in 400 ml. of diethyl oxalate at 90° C. was added with stirring 120 grams of m-chlorosulfonylbenzoyl chloride. The mixture was heated for 1/2 hour, cooled to 20° C. and the solid which separated was collected, triturated in water, ethyl acetate and dried, yielding 98 grams of product, M.P. 176-177° C.

*Coupler XXXVI: Intermediate B.—1-phenyl-3-(3-sulfonylbenzamido)-5-pyrazolone*

A mixture of 58 grams of Intermediate A above in 250 ml. of 10 percent sodium hydroxide was stirred at room temperature for 2 hours after which time the solution was acidified with concentrated hydrochloric acid whereupon a solid separated. This solid was collected, washed with water and dried, yielding 23 grams of product, M.P. dec. 292° C.

Couplers XXXVII and XXXVIII were each prepared according to the procedure given for coupler XXXVI above using the appropriate intermediates.

*Coupler XXXIX: 1-phenyl-3-(3,5-disulfonylbenzamido)-4-(4-hydroxy-2-pentadecylphenylazo) - 5 - pyrazolone dipotassium salt*

To a solution of 5 grams of 1-phenyl-3-(3,5-disulfonylbenzamido)-5-pyrazolone dipotassium salt (prepared according to the procedure given for Intermediate B, coupler XXXVI above using the appropriate intermediates) in 20 ml. of 50 percent pyridine was added at 20° C. a diazonium solution consisting of 3 grams of 4-amino-3-pentadecylphenol, 1.5 grams of isoamyl nitrite and 2 grams of concentrated hydrochloric acid in 20 ml. of n-propyl alcohol. The resultant mixture was stirred at room temperature for 12 hours after which time it was poured into 100 ml. of saturated potassium chloride solution. The solid which separated was collected, and recrystallized from 50 ml. of 60 percent ethyl alcohol, yielding the product.

Couplers XL, XLI, XLII, XLIII and XLIV were each prepared according to the procedure given for coupler XXXIX above using the appropriate intermediates.

*Coupler XLV: 1-[4-(3,5-dicarboxybenzamido)phenyl]-3-ethoxy-4-(3-octadecylcarbamylphenylthio)-5-pyrazolone*

A mixture of 7.8 grams of Intermediate H below, 25 ml. of ethyl alcohol, 15 ml. of 2 N aqueous NaOH, and 35 ml. of water was stirred at 85° C. for 15 minutes. The solution was cooled to room temperature and acidified with 1:2 concentrated HCl—water.

The solid which separated was filtered off, washed with water, acetonitrile, and recrystallized from methanol, yielding 4 grams of product, M.P. 200-202° C.

*Coupler XLV: Intermediate A.—1-(4-nitrophenyl)-3-ethoxy-5-pyrazolone*

A mixture of 31 grams of 4-nitrophenylhydrazine, 100 ml. of ethyl alcohol, and 38 grams of ethyl-β,β-diethoxyacrylate was refluxed for 1/2 hour. A solution of sodium ethoxide (prepared from 4.6 grams of sodium and 100 ml. of ethyl alcohol) was added and refluxed for another 20 minutes. This solution was acidified with glacial acetic acid and the solid which separated was filtered off, and recrystallized from 250 ml. of n-butyl alcohol, yielding 31 grams of product, M.P. 153-4° C.

*Coupler XLV: Intermediate B.—1-(4-aminophenyl)-3-ethoxy-5-pyrazolone*

A mixture of 15 grams of Intermediate A above in 150 ml. of ethyl alcohol was reduced using Pd/Charcoal at 50 p.s.i., hydrogen pressure.

The catalyst was filtered off and the solution poured into 500 ml. of water.

The product was filtered off and air dried, yielding 8.2 grams of product, M.P. 121-122° C.

*Coupler XLV: Intermediate C.—Triethyltrimesate*

A mixture of 37 grams of trimesic acid (proc. N. Dak. Acad. SC: 8, 54, (1954); CA (1955) 8898b), 100 ml. of ethyl alcohol, 50 ml. of benzene, and 1 ml. of concentrated  $H_2SO_4$  was refluxed through a 6-inch packed column surmounted by a Dean Stark water spouter for 24 hours after which time the residue was cooled and the solid which crystallized was filtered and dried.

The yield of the triester was 38 grams, M.P. 133-5° C.

*Coupler XLV: Intermediate D.—Diethyl ester of trimesic acid, (3,5-dicarbethoxybenzoic acid)*

To a solution of 147 grams of the Intermediate C above in 2 liters of ethyl alcohol was added with stirring 250 ml. of 2 N NaOH in 500 ml. of ethyl alcohol. This mixture was refluxed for 30 minutes and stirred at room temperature for 12 hours, during which time a solid separated. This solid was filtered off and recrystallized from a mixture of 500 ml. of ethyl alcohol and 500 ml. of water, yielding 80 grams of product, M.P. 153-5° C.

*Coupler XLV: Intermediate E.—3,5-dicarbethoxybenzoyl chloride*

A mixture of 300 grams of Intermediate D above and 2 liters of thionyl chloride was refluxed for 2 hours, after which time it was concentrated in vacuo.

To the residue was added 250 ml. of dry benzene and again concentrated in vacuo.

The acid chloride thus formed was used as such in preparing Intermediate F below.

*Coupler XLV: Intermediate F.—1-[4-(3,5-dicarbethoxybenzamido)phenyl]-3-ethoxy-5-pyrazolone*

A mixture of 6.6 grams of Intermediate B above and 8.5 grams of Intermediate E above and 100 ml. of dry acetonitrile was refluxed for 5 hours. The mixture was cooled to room temperature and the solid was filtered off, dried, and recrystallized from glacial acetic acid, yielding 10 grams of product, M.P. 200-201° C.

*Coupler XLV: Intermediate G.—3-octadecylcarbamylphenylsulfenyl chloride*

Into a suspension of 8 grams of 3,3'-dioctadecylcarbamylidiphenyldisulfide (Loria et al. U.S. patent application Ser. No. 154,841, filed 11-24-61, now abandoned) in 120 ml. of anhydrous carbon tetrachloride was bubbled dry chlorine gas for 1½ hours at room temperature, during which time all of the solid dissolved and a clear light yellow solution was formed. The solution was concentrated in vacuo to a volume of 50 ml. to remove excess chlorine.

This solution of the sulfenyl chloride was used as such in the following reaction (i.e., Intermediate H below).

*Coupler XLV: Intermediate H.—1-[4-(3,5-dicarbethoxybenzamido)phenyl]-3-ethoxy-4-(3-octadecylcarbamylphenylthio)-5-pyrazolone*

A mixture of Intermediate G above and 9.35 of Intermediate F in 200 ml. of dry dioxane was stirred at room temperature for 2 hours, heated to reflux for 1 hour, and concentrated in vacuo.

The residue was recrystallized from ethyl alcohol, yielding 8.5 grams of product, M.P. 156-8° C.

*Coupler XLVI: 1-(4-sulfophenyl)-3-(4-sulfoanilino)-4-(3-octadecylcarbamylphenylthio)-5-pyrazolone disodium salt*

A suspension of 25 grams of Intermediate B below in 100 ml. of ethyl alcohol and 200 ml. of 2 percent aqueous NaOH was stirred at room temperature for ½ hour, during which time all solid dissolved. The solution was cooled and acidified with 5 ml. of acetic acid and concentrated in vacuo.

The crude solid residue was recrystallized from methyl alcohol, yielding 10 grams of product, M.P. >250° C.

*Coupler XLVI: Intermediate A.—1-(4-fluorosulfonylphenyl)-3-(4-fluorosulfonylanilino)-5-pyrazolone*

To 450 ml. of fluosulfonic acid at 5° C. was added with stirring 80 grams of 1-phenyl-3-anilino-5-pyrazolone.

The resultant solution was stirred at 50° C. for 4½ hours, then poured onto 2 kg. of crushed ice. The solid was collected, washed with water, filtered, and dissolved in 2 liters of ethyl acetate. This solution was washed with 5 percent sodium bicarbonate solution, water, and saturated brine.

It was concentrated in vacuo and the residue was recrystallized from acetonitrile, yielding 36 grams of product, M.P. 290° C. decomp.

*Coupler XLVI: Intermediate B.—1-(4-fluorosulfonylphenyl)-3-(4-fluorosulfonylanilino)-4-(3-octadecylcarbamylphenylthio)-5-pyrazolone*

A mixture of Intermediate G of Coupler XLV above (prepared from 24.5 grams of the disulfide) and 25 grams of Intermediate A above in 330 ml. of dry carbon tetrachloride was stirred at 55° C. for 12 hours.

The solution was then concentrated in vacuo and the residue was recrystallized from 300 ml. of ethyl acetate yielding 25 grams of product, M.P. 209-11° C.

*Coupler XLVII: 4,4'-(4-octadecyloxybenzylidene)bis[1-phenyl-3-(3,5-disulfobenzamido)-5-pyrazolone]tetra-potassium salt*

To a refluxing solution of 5.2 grams of 1-phenyl-3-(3,5-disulfobenzamido)-5-pyrazolone dipotassium salt in 45 ml. of ethyl alcohol and 20 ml. of water was added a solution of 1.9 grams of Intermediate A below and 0.5 gram of piperidine in 35 ml. of ethyl alcohol. The solution was refluxed for ½ hour and cooled to room temperature. The solid which separated was collected, recrystallized from 90 percent ethyl alcohol, yielding 5 grams of product.

*Coupler XLVII: Intermediate A.—4-octadecyloxybenzaldehyde*

To a solution of 23 grams of sodium metal and 122 grams of 4-hydroxybenzaldehyde in 500 ml. of ethyl alcohol was added 333 grams of 1-bromooctadecane. The mixture was refluxed with stirring for 20 hours during which time a solid separated. This solid was filtered and the filtrate was concentrated in vacuo. The residual material was then distilled at 253° C. at 1 mm. pressure yielding 250 grams of product.

*Coupler XLVII:  $\alpha$ -Benzoyl- $\alpha$ -(4-hydroxy-2-pentadecylphenylazo)-4-(3-sulfobenzamido) acetanilide sodium salt*

To a solution of 4.5 grams of  $\alpha$ -benzoyl-4-(3-chlorosulfonylbenzamido) acetanilide in 12 ml. of 90 percent pyridine was added at 20° C. a diazonium mixture consisting of 3.2 grams of 4-amino-3-pentadecylphenol, 1.4 grams of isoamyl nitrite and 2 ml. of concentrated hydro-

chloric acid in 20 ml. of n-propyl alcohol. The resultant solution was stirred at room temperature for 12 hours after which time it was poured into 50 ml. of saturated sodium chloride solution. The yellow solid which separated was collected, and recrystallized twice from ethyl alcohol, yielding 2.2 grams of product.

Coupler XLIX was prepared according to the procedure given for coupler XLVII above using the appropriate intermediates.

*Coupler LI:  $\alpha$ -Benzoyl- $\alpha$ -(3-octadecylcarbamylphenylthio)-3,5-dicarboxyacetanilide*

To a mixture of 7 grams of Intermediate A below in 100 ml. of dioxane at 50° C. was added a solution of 3-octadecylcarbamylphenylsulfenyl chloride (Intermediate G of coupler XLV above, prepared from 8.1 grams

of the disulfide), in 100 ml. of dioxane. This mixture was stirred for 12 hours after which time the solution was concentrated in vacuo. A solution of the gummy residue in 100 ml. of ethyl alcohol and 13 ml. of 2 N aqueous sodium hydroxide was heated at 40° C. for 1 hour after which time it was acidified with concentrated hydrochloric acid. The solid which separated was collected and recrystallized twice from ethyl alcohol, yielding 2 grams of product, M.P. 140-142° C.

*Coupler LI: Intermediate A.— $\alpha$ -Benzoyl-3,5-dicarbomethoxyacetanilide*

To a refluxing mixture of 102 grams of ethyl  $\alpha$ -benzoylacetate and 5 grams of sodium acetate in 100 ml. of xylene was added 105 grams of dimethyl 5-aminoisophthalate. The resulting solution was refluxed under a steam condenser for 3 hours after which time it was concentrated to  $\frac{1}{2}$  the original volume and cooled to room temperature. The solid which separated was collected and recrystallized from methyl alcohol, yielding 40 grams of product, M.P. 165-167° C.

The following examples illustrate typical embodiments of the invention.

*Example 1*

A color film having the structure substantially as shown in FIG. 1 was prepared by coating a subbed cellulose acetate film support successively with the following layers which correspond to the numbered layers in FIG. 1.

*Layer 11.*—A gelatino silver chloride emulsion coated at 40 mg. silver per square foot and 100 mg. gelatin per square foot and containing  $2.7 \times 10^{-7}$  gm. zinc sulfide (nuclei) per square foot, 50 mg. 1-hydroxy-4-(3-octadecylcarbamylphenylthio) - N - ethyl-3',5'-dicarboxy-2-naphthanilide per square foot and 15 mg. 2-octadecyl-5-sulfohydroquinone potassium salt per square foot. The phenolic DDR coupler of this layer yields a diffusible indoaniline cyan dye image upon reaction with oxidized color developing agent in the uninhibited areas of layer 11.

*Layer 12.*—A red-sensitive gelatino-silver bromoiodide emulsion coated at 75 mg. silver per square foot and 100 mg. gelatin per square foot and containing 60 mg. of the DIR compound, 2-{4-[3-(4-tert-amyl - x - sulfophenoxy) benzamido]phenethyl}-x-(1-phenyl-5-tetrazolylthio) - hydroquinone (Compound I), per square foot. The DIR compound of this layer and of layers 15 and 18, cross oxidizes with oxidized color developing agent, in the region of exposure, to form a quinone which compound releases the tetrazolylthio radical to yield the corresponding mercaptan which is effective to inhibit the development of the adjacent nucleated silver halide of layers 11, 14 and 17 respectively.

*Layer 13.*—A gelatino-silver iodide emulsion coated at 50 mg. silver per square foot and 100 mg. gelatin per square foot and containing 30 mg. of the nondiffusing magenta colored filter dye, 1-hydroxy-4'-(4-tert-butylphenoxy)-4-phenylazo-2-naphthamide, per square foot and 30 mg. 2-octadecyl-5-sulfo-hydroquinone potassium salt per square foot. The silver iodide of this layer and of layer 16 serves to prevent upward diffusion of the mercaptan from layers 12 and 15.

*Layer 14.*—A gelatino-silver chloride emulsion coated at 40 mg. silver per square foot and 100 mg. gelatin per square foot and containing  $5.5 \times 10^{-6}$  gm. zinc sulfide (nuclei) per square foot, 50 mg. of 1-phenyl-3-(3,5-dissulfonylbenzamido) - 4-(2-hydroxy-4-n-pentadecylphenylazo)-5-pyrazolone dipotassium salt per square foot and 15 mg. 2-octadecyl-5-sulfo-hydroquinone potassium salt per square foot. This 5-pyrazolone DDR coupler yields a diffusible magenta azomethine dye image in the process.

*Layer 15.*—A green-sensitive gelatino-silver bromoiodide emulsion coated at 0.075 grams silver per square

foot, 100 mg. gelatin per square foot, and 60 mg. of DIR compound, 2-{4-[3-(4-tert-amyl-x-sulfophenoxy)benzamido]phenethyl} - x - (1-phenyl-5-tetrazolylthio)hydroquinone (Compound I), per square foot.

*Layer 16.*—A gelatino-silver iodide emulsion containing 50 mg. silver per square foot and 100 mg. gelatin per square foot and also 66 mg. 1-(2,4,6-trichlorophenyl)-3-{3-[ $\alpha$ -(2,4-di-tert-amylphenoxy)acetamido]benzamido}-4-(p-methoxyphenylazo)-5-pyrazolone per square foot and 30 mg. 2-octadecyl-5-sulfohydroquinone potassium salt per square foot. The yellow pyrazolone coupler of this layer serves as a light filter to confine the blue image exposure to layer 18.

*Layer 17.*—A gelatino-silver chloride emulsion coated at 50 mg. silver per square foot and 100 mg. gelatin per square foot and containing also  $1.1 \times 10^{-6}$  gm. zinc sulfide (nuclei) per square foot, 100 mg.  $\alpha$ -benzoyl- $\alpha$ -(3-octadecylcarbamylphenylthio) - 3,5 - dicarboxyacetanilide per square foot and 15 mg. 2-octadecyl-5-sulfo-hydroquinone potassium salt per square foot. The DDR coupler of this layer yields a diffusible yellow azo methine dye image in the process.

*Layer 18.*—A blue-sensitive gelatino-silver bromoiodide emulsion coated at 0.075 gram silver per square foot and 100 mg. gelatin per square foot and containing in addition, 30 mg. of the DIR compound, 2-{4-[3-(4-tert-amyl - x - sulfophenoxy)benzamido]phenethyl} - x - (1-phenyl-5-tetrazolylthio)hydroquinone (Compound I), per square foot.

The resulting element was exposed to a colored subject and immersed with a paper receiving sheet having a gelatin layer containing a mordant such as cetyl trimethyl ammonium bromide in the following color developing solution and pressed for about 5 minutes at 85° F. into contact with the paper reception sheet.

|                                                                              |                     |       |
|------------------------------------------------------------------------------|---------------------|-------|
| Ascorbic acid                                                                | mg                  | 200.0 |
| 4-amino-N-ethyl-N- $\beta$ -hydroxyethyl aniline sulfate                     | g                   | 4.0   |
| 4-amino-N-ethyl-N- $\beta$ -methylsulfonamido-ethyl-2-methyl aniline sulfate | g                   | 1.0   |
| Na <sub>2</sub> CO <sub>3</sub> · H <sub>2</sub> O                           | g                   | 40.0  |
| Aminoethanol                                                                 | ml                  | 2.2   |
| Potassium bromide                                                            | mg                  | 500.0 |
| Sodium thiosulfate (pentahydrate)                                            | mg                  | 200.0 |
| 6-nitrobenzimidazole nitrate                                                 | mg                  | 5.0   |
| H <sub>2</sub> O to 1 liter                                                  | pH 11.0 (adjusted). |       |

As a result, the exposed silver halide in layers 12, 15 and 19 develops and the DIR compound therein cross-oxidizes with oxidized color developing agent obtaining in the reaction thereby releasing a development inhibiting mercaptan that inhibits development of adjacent areas of the nucleated emulsion layers 11, 14 and 17 respectively. The residual developer solution migrates to the positive areas of layers 11, 14 and 17, causing physical development to proceed and diffusible cyan, magenta and yellow dyes to be produced which transfer by diffusion imagewise and in register to the mordanted receiving sheet to provide a multicolor positive reproduction of the original subject.

*Example 2*

A color film having the structure substantially as shown in FIG. 1 was prepared by coating on a cellulose acetate film support successively with the following layers which correspond to the numbered layers in FIG. 1:

*Layer 11.*—A gelatino-silver thiocyanate emulsion coated at 30 mg. silver per square foot and 100 mg. gelatin per square foot and containing  $2.7 \times 10^{-7}$  grams zinc sulfide (nuclei) per square foot, 50 mg. 1-hydroxy-4-(3-n-octadecylcarbamyl-phenylthio) - N - ethyl - 3',5'-dicarboxy-2-naphthamide per square foot and 15 mg. 2-octadecyl-5-sulfohydroquinone potassium salt per square foot. The phenolic DDR coupler of this layer yields a diffusible indoaniline cyan dye image upon reac-

tion with the oxidized color developing agent in the uninhibited areas of layer 11.

*Layer 12.*—A red-sensitive gelatino-silver bromoiodide emulsion coated at 0.112 grams silver per square foot and 160 mg. gelatin per square foot and containing 45 mg. of the DIR compound, 2-[4-[3-(4-tert-amyl-x-sulfophenoxy)benzamido]phenethyl]-x-(1-phenyl-5-thiazolylthio)hydroquinone (Compound I), per square foot.

The DIR compound of this layer, and of layers 15 and 18, cross oxidizes with oxidized color developing agent, in the region of exposure, to release the tetrazolylthio radical which is effective to inhibit the development of the adjacent nucleated silver salt of layers 11, 14 and 17 respectively.

*Layer 13.*—A gelatino-silver iodide emulsion coated at 50 mg. silver per square foot and 80 mg. gelatin per square foot and containing 22.5 mg. of the nondiffusing magenta colored filter dye, 1-hydroxy-4'-(4-tert-butylphenoxy)-4-phenylazo-2-naphthamide, per square foot and 30 mg. 2-octadecyl-5-sulfohydroquinone potassium salt per square foot. The silver iodide of this layer and of layer 16 serves to prevent upward diffusion of the mercaptan from layers 12 and 15.

*Layer 14.*—A gelatino-silver thiocyanate emulsion coated at 49 mg. silver per square foot and 100 mg. gelatin per square foot and containing  $5.4 \times 10^{-6}$  gm. zinc sulfide (nuclei) per square foot, 50 mg. of 1-phenyl-3-(3,5-disulfobenzamido)-4-(2-hydroxy-4-n-pentadecylphenylazo)-5-pyrazolone dipotassium salt per square foot and 15 mg. 2-octadecyl-5-sulfohydroquinone potassium salt per square foot. This 5-pyrazolone DDR coupler yields a diffusible magenta azomethine dye image in the process.

*Layer 15.*—A green-sensitive gelatino-silver bromoiodide emulsion coated at 0.075 grams silver per square foot, 100 mg. gelatin per square foot, and 30 mg. of the DIR compound, 2-[4-[4-tert-amyl-x-sulfophenoxy]benzamido]phenethyl]-x-(1-phenyl-5-tetrazolylthio)hydroquinone, per square foot.

*Layer 16.*—A gelatino-silver iodide emulsion containing 50 mg. silver per square foot and 100 mg. gelatin per square foot and 100 mg. gelatin per square foot and also 66 mg. 1-(2,4,6-trichlorophenyl)-3-[3-[ $\alpha$ -(2,4-di-tert-aminophenoxy)acetamido]benzamido]-4-(p-methoxy-2-octadecyl-5-sulfohydroquinone potassium salt per square foot and 30 mg. 2-octadecyl-5-sulfohydroquinone potassium salt per square foot. The yellow pyrazolone coupler of this layer serves as a light filter to confine the blue image exposure to layer 18.

*Layer 17.*—A gelatino-silver thiocyanate emulsion coated at 40 mg. silver per square foot and 100 mg. gelatin per square foot and containing also  $7.2 \times 10^{-7}$  grams zinc sulfide (nuclei) per square foot, 100 mg.  $\alpha$ -benzoyl- $\alpha$ -(3-octadecylcarbamyl-phenylthio)-3,5-dicarboxyacetanilide per square foot and 15 mg. 2-octadecyl-5-sulfohydroquinone potassium salt per square foot. The DDR coupler of this layer yields a diffusible yellow azomethine dye image in the process.

*Layer 18.*—A blue-sensitive gelatino-silver bromoiodide emulsion coated at 75 mg. silver per square foot and 100 mg. gelatin per square foot and containing, in addition, 30 mg. of the DIR compound, 2-[4-[3-(4-tert-amyl-x-sulfophenoxy)benzamido]phenethyl]-x-(1-phenyl-5-tetrazolylthio)hydroquinone, per square foot.

The resulting element was exposed to a colored subject and immersed with a paper receiving sheet having a gelatin layer containing a mordant such as cetyl trimethyl ammonium bromide in the following color developing solution and placed for about 5 minutes at 85° F. into contact with the paper reception sheet.

|                                                          |    |     |
|----------------------------------------------------------|----|-----|
| Ascorbic acid                                            | mg | 200 |
| 4-amino-N-ethyl-N- $\beta$ -hydroxyethyl aniline sulfate | g  | 5   |
| Na <sub>2</sub> CO <sub>3</sub> · H <sub>2</sub> O       | g  | 40  |

|                                   |    |                     |
|-----------------------------------|----|---------------------|
| N,N-diethyl-1,3-propanediamine    | ml | 1                   |
| Sodium thiosulfate (pentahydrate) | mg | 100                 |
| H <sub>2</sub> O to 1 liter       |    | pH 11.0 (adjusted). |

As a result, the exposed silver halide in layers 12, 15 and 18 develops and the DIR compound therein cross-oxidizes with the oxidized color developing agent obtained in the reaction thereby releasing the development inhibiting mercaptan that inhibits development of adjacent areas of the nucleated silver thiocyanate emulsion layers 11, 14 and 17 respectively. The residual developer solution migrates to the positive areas of layers 11, 14 and 17 causing physical development to proceed and diffusible cyan, magenta and yellow dyes to be produced which transfer by diffusion imagewise and in register to the mordanted receiving sheet to provide a multicolor positive reproduction of the original subject thereon.

#### Example 3

20 A color film having the structure substantially as shown in FIG. 2 was prepared by coating a subbed cellulose acetate film support successively with the following layers which correspond to the numbered layers of FIG. 2:

25 *Layer 21.*—A fogged gelatino-silver chlorobromoiodide emulsion containing one mole of silver, 8,400 cc. of 1 percent aqueous solution of the magna-forming DDR coupler, 1-phenyl-3-(3,5-disulfobenzamido)-4-(4-octadecyloxyphenylazo)-5-pyrazolone disodium salt, 740 cc. of 7.5 percent saponin in water, 134 cc. of 2.7 percent mucochloric acid in water and water to make 22,100 grams was coated on the support so that the resulting layer contained 30 mg. of silver per square foot, 30 mg. of the DDR coupler per square foot and 184 mg. of gelatin per square foot.

35 *Layer 22.*—A gelatino-silver chlorobromoiodide emulsion sensitized to green light and containing one mole of the silver halide, the DIR compound, 2-[4-(3,5-disulfobenzamido)phenethyl]-x-(1-phenyl-5-tetrazolylthio)hydroquinone Disodium Salt Dihydrate (Compound V), dispersed in aqueous gelatin solution, 400 cc. of 7.5 percent saponin, 73 cc. of 2.7 percent mucochloric acid and water to make 12,000 grams was coated to give 62 mg. of silver per square foot, 91 mg. of the DIR compound per square foot and 214 mg. of gelatin per square foot.

40 *Layer 23.*—A gelatino-silver chloride emulsion containing one mole of silver, 2.6 cc. of 7.5 percent saponin, 43 cc. of 2.7 percent mucochloric acid and water to make 6,480 grams was coated in a layer having 100 mg. of silver per square foot and 200 mg. of gelatin per square foot.

45 *Layer 24.*—This layer is substantially the same as layer 21 except that the fogged silver halide emulsion contained the cyan-forming DDR coupler, 2-(3,5-disulfobenzamido)-5-methyl-4-(4-octadecyloxyphenylazo)phenol dipotassium salt, in lieu of the magna-forming DDR coupler, the coupler being coated to obtain a layer having 87 mg. of the coupler per square foot.

50 *Layer 25.*—This layer is substantially the same as layer 22 except that one mole of a gelatino-silver chlorobromoiodide emulsion sensitive to red light was utilized in lieu of the green-sensitive silver halide emulsion.

55 *Layer 26.*—This layer is substantially the same as layer 23 except that sufficient Carey Lea silver is added to obtain a coverage of 4.6 mg. per square foot.

60 *Layer 27.*—This layer is substantially the same as layer 21 except that the fogged silver halide emulsion containing the yellow-forming DDR coupler, 1-hydroxy-4-(2,4-dinitrophenylthio)-N-[ $\delta$ -(2,4-di-tert-aminophenoxy)butyl]-2-naphthamide, was used in lieu of the magenta-forming DDR coupler.

65 *Layer 28.*—This layer is substantially the same as layer 22 except that one mole of gelatino-silver chlorobromide emulsion sensitive to blue light was used in lieu of the green-sensitive silver halide emulsion.

70 *Layer 29.*—This is a protective gelatin layer at a coverage of 50 mg. of gelatin per square foot.

The fogged silver halide emulsions were prepared by exposing the emulsions to a 40-watt bulb at 60 inches for 30 seconds. The resulting photographic element was exposed to a colored subject and immersed with a paper receiving sheet having a gelatin layer containing a mordant such as dimethyl- $\beta$ -hydroxy-ethyl- $\alpha$ -(octadecylamido)-propyl ammonium dihydrogen phosphate in the following color developing solution and squeegeed together for about 5 minutes at 85° F.

|                                        |     |    |
|----------------------------------------|-----|----|
| Sodium carbonate                       | g.  | 20 |
| Sodium hexametaphosphate               | g.  | 20 |
| Benzyl alcohol                         | cc. | 10 |
| 3-Acetamido-4-amino-N,N-diethylaniline | g.  | 2  |
| Water to one liter, pH adjusted to 11. |     | 15 |

As a result, the exposed silver halide in layers 22, 25 and 28 develops and the DIR compound in layers 22, 25 and 28 contiguous thereto cross-oxidizes with oxidized color developing agent formed in the development of the exposed silver halide, thereby releasing a diffusible mercaptan that inhibits development in adjacent negative areas in the fogged emulsion layers 21, 24 and 27. The residual developer solution migrates to the positive areas of layers 21, 24 and 27, and proceeds to develop these fogged layers to form diffusible magenta, cyan and yellow dyes which transfer by diffusion imagewise and in register to the mordanted receiving sheet to provide a multicolor positive reproduction of the original subject.

#### Example 4

The color films described in Examples 1, 2 and 3 above, respectively, were also processed in a manner similar to that described in the above examples using the following developer releases the tetrazolylthio radical to yield the corresponding mercaptan which is effective to inhibit the development of the adjacent nucleated silver halide of Layers 11, 14 and 17 respectively.

*Layer 13.*—A gelatino silver iodide emulsion coated at 50 mg. silver per square foot and 100 mg. gelatin per square foot and containing 30 mg. 2-octadecyl-5-sulfohydroquinone potassium salt per square foot. The silver iodide of this layer and of Layer 16 serves to prevent upward diffusion of the mercaptan from Layers 12 and 15.

*Layer 14.*—A gelatino silver chloride emulsion coated at 40 mg. silver per square foot and 100 mg. gelatin per square foot and containing  $5.5 \times 10^{-6}$  gm. zinc sulfide (nuclei) per square foot, 70 mg. of 1-(2,5-dichlorophenyl) - 3 - [3 - (4-tert-amylphenoxy)-benzamido]-5-pyrazolone per square foot and 15 mg. 2-octadecyl-5-sulfohydroquinone potassium salt per square foot. This 5-pyrazolone coupler yields a non-diffusible magenta azomethine dye image in the process.

*Layer 15.*—A green-sensitive gelatino silver bromoiodide emulsion coated at 75 mg. silver per square foot, 100 mg. gelatin per square foot and 60 mg. of DIR compound, 2 - {4 - [3 - (4-tert-amylphenoxy)-benzamido]phenethyl}-x - (1-phenyl-5-tetrazolylthio)hydroquinone (Compound I), per square foot.

*Layer 16.*—A gelatino silver iodide emulsion containing 50 mg. silver per square foot and 100 mg. gelatin per square foot and also 10 mg. Carey Lea silver per square foot and 30 mg. 2-octadecyl-5-sulfohydroquinone potassium salt per square foot. The yellow Carey Lea silver of this layer serves as a light filter to confine the blue image exposures to Layer 18.

*Layer 17.*—A gelatino silver chloride emulsion coated at 50 mg. silver per square foot and 100 mg. gelatin per square foot and containing also  $1.1 \times 10^{-6}$  gm. zinc sulfide (nuclei) per square foot, 100 mg.  $\alpha$ -{4-[ $\alpha$ -(2,4-ditert-amylphenoxy)acetamido]benzoyl} - 2 - methoxyacetanilide per square foot and 15 mg. 2-octadecyl-5-sulfohydroquinone potassium salt per square foot. The coupler of this layer yields non-diffusible yellow azomethine dye image in the process.

*Layer 18.*—A blue-sensitive gelatino silver bromoiodide emulsion coated at 75 mg. silver per square foot and 100 mg. gelatin per square foot and containing in addition, 30 mg. of the DIR compound, 2-{4-[3-(4-tert-amyl-x-sulfophenoxy)benzamido]phenethyl} - x - (1 - phenyl-5-tetrazolylthio)hydroquinone (Compound I), per square foot.

The resulting element was exposed to a colored subject and was then treated in a color developer at 75° F. for 7 minutes having the following composition:

|                                                                             |     |       |
|-----------------------------------------------------------------------------|-----|-------|
| Sodium carbonate                                                            | g.  | 20    |
| Sodium hexametaphosphate                                                    | g.  | 20    |
| Benzyl alcohol                                                              | cc. | 10    |
| 3-Acetamido-4-amino-N,N-diethylaniline                                      | g.  | 2     |
| Water to one liter, pH adjusted to 11.                                      |     | 15    |
| Ascorbic acid                                                               | mg. | 200.0 |
| 4-amino-N-ethyl-N- $\beta$ -hydroxyethyl aniline sulfate                    | g.  | 4.0   |
| 4-amino-N-ethyl-N- $\beta$ -methylsulfonamidoethyl-2-methyl aniline sulfate | g.  | 1.0   |
| Na <sub>2</sub> CO <sub>3</sub> · H <sub>2</sub> O                          | g.  | 40.0  |
| Na <sub>2</sub> SO <sub>3</sub>                                             | g.  | 15.0  |
| Aminoethanol                                                                | ml. | 2.2   |
| Potassium bromide                                                           | mg. | 500.0 |
| Sodium thiosulfate (pentahydrate)                                           | mg. | 200.0 |
| 6-nitrobenzimidazole nitrate                                                | mg. | 5.0   |
| H <sub>2</sub> O to 1.0 liter, pH to 11.0 (adjusted).                       |     |       |

The element was then thoroughly washed with water and treated in a clearing and fixing bath having the following composition:

|                          |    |       |
|--------------------------|----|-------|
| Sodium thiosulfate       | g. | 150.0 |
| Sodium bisulfite         | g. | 20.0  |
| Water to make 1.0 liter. |    |       |

The element was then treated in a bleach bath having the following composition:

|                          |    |      |
|--------------------------|----|------|
| Potassium dichromate     | g. | 5.0  |
| Potassium ferricyanide   | g. | 70.0 |
| Potassium bromide        | g. | 20.0 |
| Water to make 1.0 liter. |    |      |

The element was again washed and once again treated with the clearing and fixing bath identified above. The element was again washed and treated in a stabilizing bath having the following composition:

|                               |     |     |
|-------------------------------|-----|-----|
| Formaldehyde (37% by weight)  | ml. | 7.0 |
| Dispersing agent <sup>1</sup> | g.  | 0.5 |
| aWt to make 1.0 liter.        |     |     |

<sup>1</sup> Such as Triton-X 100, i.e., an alkylaryl poly ether alcohol (octylphenoxy polyethoxy ethanol).

As a result, the exposed silver halide in layers 12, 15 and 18 develops and the DIR compound therein cross-oxidizes with oxidized color developing agent obtained in the reaction, thereby releasing a development inhibiting mercaptan that inhibits development of adjacent areas of the nucleated emulsion layers 11, 14 and 17 respectively. The residual developer solution migrates to the positive areas of layers 11, 14 and 17, causing physical development to proceed and non-diffusible cyan, magenta and yellow dyes to be produced in the respective layers to provide a multicolor positive reproduction of the original subject.

The invention has been described in detail with particular reference to preferred embodiments thereof, but it will be understood that variations and modifications can be effected within the spirit and scope of the invention as described hereinabove and as defined in the appended claims.

I claim:

1. A color photographic process for treating an exposed photographic element containing latent negative image regions and having at least two Color-Forming Units in layers sensitive to different regions of the visible spectrum and a barrier layer separating each of said Color-Forming Units comprising a hydrophilic colloid containing a water-insoluble reactant capable of forming a water-in-

soluble salt with mercaptans, each of said Color-Forming Units comprising

- (1) a light-sensitive emulsion of a hydrophilic colloid and a silver halide;
- (2) an emulsion of a hydrophilic colloid and a water-insoluble metal salt developable to substantial density with a color developing agent without exposure to light;
- (3) a nondiffusible dye forming coupler contiguous to said water-insoluble metal salt of said developable emulsion and which coupler forms an image dye on reaction with an oxidized color developing agent;

which comprises treating said exposed photographic element with a photographic alkaline color developing solution containing an aromatic primary amino developing agent so that in each of said Color-Forming Units said silver halide in said negative image regions of said light-sensitive emulsion is developed with said developing agent in the presence of a non-color forming development inhibitor-releasing hydroquinone compound that reacts with oxidized color developing agent to form a diffusible mercaptan development inhibitor in said negative image regions, reacting said development inhibitor-releasing hydroquinone compound with resulting oxidized developing agent and forming a diffusible mercaptan development inhibitor, said diffusible mercaptan development inhibitor thereafter diffusing to said developable emulsion and inhibiting development in regions corresponding to said negative image regions, said barrier layer preventing said diffusible mercaptan development inhibitor formed in one Color-Forming Unit from diffusing to another Color-Forming Unit by forming an insoluble salt with mercaptans diffusing to said barrier layer, said developable emulsion thereafter being developed with said developing agent in the presence of said image dye forming coupler that reacts with resulting oxidized developing agent to form a dye image in regions not inhibited against development by said mercaptan development inhibitor, said image dye forming coupler having a formula selected from the group consisting of

BALL-COUP,  
DYE-LINK-(COUP-BALL)<sub>n</sub>  
and  
BALL-LINK-(COUP-SOL)<sub>n</sub>  
BALL-LINK-COUP

and said development inhibitor-releasing hydroquinone compound having the formula



wherein

- (1) DYE is a dye radical exhibiting selective absorption in the visible spectrum and containing an acidic solubilizing group,
- (2) LINK is a connecting radical selected from the group consisting of an azo radical, a mercuri radical, an oxy radical, an alkylidene radical, a monothio radical, a dithio radical and an azoxy radical,
- (3) —S—is a monothio connecting radical,
- (4) COUP is a photographic coupler radical selected from the group consisting of a 5-pyrazolone coupler radical, a phenolic coupler radical and an open-chain ketomethylene coupler radical, said COUP being substituted in the coupling position with a member

selected from the group consisting of hydrogen, halogen, sulfonic acid and any one of said connecting radicals,

- (5) BALL is a photographically inert organic ballasting radical of such molecular size and configuration as to render said couplers and said hydroquinone compound nondiffusible,
- (6) SOL is selected from the group consisting of a hydrogen atom and an acidic solubilizing group when said developing agent contains an acidic solubilizing group, and SOL is an acidic solubilizing group when said developing agent is free of an acidic solubilizing group,
- (7) n is an integer of 1 to 2 when said LINK is an alkylidene radical, and n is 1 when said LINK is a radical selected from the group consisting of an azo radical, a mercuri radical, an oxy radical, a monothio radical, a dithio radical and an azoxy radical,
- (8) RAD is a photographically inert diffusible radical that forms a mercaptan with said monothio connecting radical,
- (9) R is selected from the group consisting of a hydrogen atom and an alkaline splittable acyl masking group, and
- (10) R<sub>1</sub> is selected from the group consisting of a hydrogen atom and an alkaline splittable acyl masking group.

2. The process as described in claim 1 wherein the developable emulsion is an emulsion of a hydrophilic colloid and a silver halide that is fogged so that it can be developed to substantial density without exposure to light with a photographic alkaline color developing solution containing an aromatic primary amino developing agent.

3. The process as described in claim 1 wherein the developable emulsion is an emulsion of a hydrophilic colloid and a silver halide containing physical development nuclei.

4. A color photograph diffusion transfer process for treating an exposed photographic element containing latent negative image regions and having superposed on a photographic support three Color-Forming Units in layers sensitive to red, green and blue light respectively, and a barrier layer separating each of said Color-Forming Units comprising a hydrophilic colloid containing a silver halide; each of said Color-Forming Units comprising

- (1) a light-sensitive emulsion layer of a hydrophilic colloid and a silver halide,
- (2) a nondiffusible and non-color forming development inhibitor-releasing hydroquinone compound, contiguous to said silver halide of said light-sensitive emulsion layer, that releases a diffusible mercaptan development inhibitor on reaction with an oxidized color developing agent,
- (3) a developable emulsion layer of a hydrophilic colloid and a water-insoluble silver salt developable to substantial density without exposure to light with a color developing agent, and
- (4) a nondifusible acid dye-releasing coupler capable of forming a diffusible acid dye contiguous to said water-insoluble silver salt of said developable emulsion layer on reaction with an oxidized color developing agent, said acid dye-releasing coupler releasing a diffusible yellow acid dye when said light-sensitive emulsion layer is sensitive to blue light, a diffusible magenta dye when said light-sensitive emulsion layer is sensitive to green light and a diffusible cyan dye when said light-sensitive emulsion layer is sensitive to red light;

70 which comprises treating said exposed photographic element with a photographic alkaline color developing solution containing an aromatic primary amino developing agent so that in each of said Color-Forming Units, silver halide in said negative image regions of said light-sensitive emulsion layer is developed with said developing

agent and said development inhibitor-releasing hydroquinone compound, contiguous to the silver halide, reacts with resulting oxidized developing agent to form a diffusible mercaptan development inhibitor in said negative image regions, said diffusible mercaptan development inhibitor thereafter diffusing to said developable emulsion layer and inhibiting development in regions corresponding to said negative image regions, said barrier layers preventing said diffusible mercaptan development inhibitor formed in one Color-Forming Unit from diffusing to another Color-Forming Unit by forming an insoluble silver salt with mercaptans diffusing to said barrier layers, said developable emulsion layer thereafter being developed with said developing agent and said acid dye-releasing coupler contiguous to said water-insoluble silver salt in said developable emulsion layer reacting with resulting oxidized developing agent to form a diffusible acid dye in regions not inhibited against development by said mercaptan development inhibitor, and said diffusible acid dye diffusing imagewise in register to a juxtaposed reception layer containing a mordant for acid dyes; said acid dye-releasing coupler having a formula selected from the group consisting of

DYE-LINK-(COUP-BALL)<sub>n</sub>

and

BALL-LINK-(COUP-SOL)<sub>n</sub>,

and said development inhibitor-releasing hydroquinone compound having the formula



wherein

- (1) DYE is a dye radical exhibiting selective absorption in the visible spectrum and containing an acidic solubilizing group,
- (2) LINK is a connecting radical selected from the group consisting of an azo radical, a mercuri radical, a n oxyradical, an alkylidene radical, a monothio radical, a dithio radical and an azoxy radical,
- (3) —S— is monothio connecting radical,
- (4) COUP is a photographic coupler selected from the group consisting of a 5-pyrazolone coupler radical, a phenolic coupler radical and an open-chain ketomethylene coupler radical, said COUP being substituted in the coupling position with one of said connecting radicals,
- (5) BALL is a photographically inert organic ballasting radical of such molecular size and configuration as to render said couplers and said hydroquinone nondiffusible,
- (6) SOL is selected from the group consisting of a hydrogen atom and an acidic solubilizing group when said developing agent contains an acidic solubilizing group, and SOL is an acidic solubilizing group when said developing agent is free of an acidic solubilizing group,
- (7) n is an integer of 1 to 2 when said LINK is an alkylidene radical, and n is 1 when said LINK is a radical selected from the group consisting of an azo radical, a mercuri radical, an oxy radical, a monothio radical, a dithio radical and an azoxy radical,
- (8) RAD is a photographically inert diffusible radical

that forms a mercaptan with said monothio connecting radical,

(9) R is selected from the group consisting of a hydrogen atom and an alkaline splittable acyl masking group, and

(10) R<sub>1</sub> is selected from the group consisting of a hydrogen atom and an alkaline splittable acyl masking group.

5 5. The process as described in claim 4 wherein the reception layer is a receiving sheet separate from the photographic element and wherein said receiving sheet is wetted with the developing solution substantially concurrently with the photographic element, pressed in superposed relation to the emulsion side of the photographic element, and after the diffusible acid dyes have diffused 10 imagewise thereto, stripped from the photographic element.

10 6. A color photographic diffusion transfer process for treating an exposed photographic element containing latent negative image regions and having superposed on a photographic support three Color-Forming Units in layers sensitive to red, green and blue light respectively, the said Color-Forming Unit sensitive to blue light being furthest from said support and being separated from the other of said Color-Forming Units by a barrier layer comprising a hydrophilic colloidal substrate containing a yellow filter material and a silver halide less sensitive to light than said Color-Forming Units, and the said Color-Forming Units sensitive to red and green light respectively being 15 separated by a barrier layer comprising a hydrophilic colloidal substrate containing a silver halide less sensitive to light than said Color-Forming Units; each of said Color-Forming Units comprising

20 (1) a light-sensitive emulsion layer of a hydrophilic colloid and a silver halide,

25 (2) a nondiffusible and non-color forming development inhibitor-releasing hydroquinone compound contiguous to said silver halide of said light-sensitive emulsion layer that releases a diffusible mercaptan development inhibitor on reaction with an oxidized color developing agent,

30 (3) a developable emulsion layer of a hydrophilic colloid and a water-insoluble silver salt developable to substantial density without exposure to light with a color developing agent and positioned closer to said support than said light-sensitive layer, and

35 (4) a nondiffusible acid dye-releasing coupler capable of forming a diffusible acid dye complementary to the color of the spectral sensitivity of the light-sensitive emulsion layer on reaction with an oxidized color developing agent contiguous to said water-insoluble silver salt of said developable emulsion;

40 which comprises treating said exposed photographic element with a photographic alkaline color developing solution containing an aromatic primary amino developing agent so that in each of said Color-Forming Units silver halide in said negative image regions of said light-sensitive emulsion layer is developed with said developing agent and said development inhibitor-releasing hydro-

45 quinone compound contiguous to the silver halide reacts with resulting oxidized developing agent to form a diffusible mercaptan development inhibitor in said negative image regions, said diffusible mercaptan development inhibitor thereafter diffusing to said developable emulsion layer and inhibiting development in regions corresponding to said negative image regions, said barrier layers preventing said diffusible mercaptan development inhibitor formed in one Color-Forming Unit from diffusing to another Color-Forming Unit by forming an insoluble silver

50 salt with mercaptans diffusing to said barrier layers, said developable emulsion layer thereafter being developed with said developing agent and said acid dye-releasing coupler contiguous to said water-insoluble silver salt in said developable emulsion layer reacting with resulting 55 oxidized developing agent to form a diffusible acid dye in

regions not inhibited against development by said mercaptan development inhibitor, and said diffusible acid dye diffusing imagewise in register to a juxtaposed reception layer containing a mordant for acid dyes; said acid dye-releasing coupler having the formula

5

BALL-LINK-COUP-SOL,

and said development inhibitor-releasing hydroquinone compound having the formula

10



15

20

25

wherein

- (1) LINK is a connecting radical selected from the group consisting of an azo radical, an oxy radical and a monothio radical,
- (2) —S— is a monothio connecting radical,
- (3) COUP is a photographic coupler radical selected from the group consisting of a 5-pyrazolone coupler radical, a phenolic coupler radical and an open-chain ketomethylene coupler radical, said COUP being substituted in the coupling position with one of said connecting radicals,
- (4) BALL is a photographically inert organic ballasting radical of such molecular size and configuration as to render said couplers and said hydroquinone compound nondiffusible,
- (5) SOL is selected from the group consisting of a hydrogen atom and an acidic solubilizing group when said developing agent contains an acidic solubilizing group, and SOL is an acidic solubilizing agent when said developing agent is free of an acidic solubilizing group,
- (6) RAD is a photographically inert diffusible radical that forms a mercaptan with said monothio connecting radical,
- (7) R is selected from the group consisting of a hydrogen atom and an alkaline splitable acyl masking group, and
- (8) R<sub>1</sub> is selected from the group consisting of a hydrogen atom and an alkaline splitable acyl masking group.

7. The process as described in claim 6 wherein the developable emulsion layer is an emulsion of a hydrophilic colloid and silver thiocyanate containing physical development nuclei.

8. The process as described in claim 6 wherein the developable emulsion layer is an emulsion of a hydrophilic colloid and silver cyanide containing physical development nuclei.

9. The process as described in claim 6 wherein the developable emulsion layer is an emulsion of a hydrophilic colloid and a silver halide fogged so that it can be developed to a substantial density without exposure to light with a photographic alkaline color developing solution containing an aromatic primary amino developing agent.

10. The process as described in claim 6 wherein the developable emulsion layer is an emulsion of a hydrophilic colloid and a silver halide containing zinc sulfide physical development nuclei.

11. The process as described in claim 4 wherein
- (A) the development inhibitor releasing hydroquinone developer has the following general formula:



wherein

- (1) BALL is a photographically inert organic ballasting radical of such molecular size and configuration as to render said couplers and said hydroquinone compound nondiffusible,
  - (2) SOL is selected from the group consisting of a hydrogen atom and an acidic solubilizing group when said developing agent contains an acidic solubilizing group, and SOL is an acidic solubilizing agent when said developing agent is free of an acidic solubilizing group,
  - (3) —S— is a monothio connecting radical,
  - (4) RAD is a photographically inert diffusible radical that forms a mercaptan with said monothio connecting radical,
  - (5) R is selected from the group consisting of a hydrogen atom and an alkaline splitable acyl masking group; and
  - (6) R<sub>1</sub> is selected from the group consisting of a hydrogen atom and an alkaline splitable acyl masking group.
- (B) The nondiffusible acid dye-releasing coupler releasing a diffusible yellow acid dye is selected from the group consisting of
- (1)  $\alpha$  - benzoyl -  $\alpha$  - (3-octadecylcarbamylphenylthio)-3,5-dicarboxyacetanilide,
  - (2) 2-(3,5 - disulfobenzamido) - 5 - methyl-4-(4-octadecyloxyphenylazo)phenyl dipotassium salt,
  - (3) 1-hydroxy-4-(2,4-dinitrophenylthio) - N - [ $\delta$ -(2,4 - di-t-amylphenoxy)butyl]-2-naphthamide, and
  - (4) 1-hydroxy-4-[4-(1-sulfophenyl - 3 - methylpyrazolyl)azo] - 3 - sulfophenylazo)-N-[ $\delta$ -(2,4-di-t-amylphenoxy)butyl]-2-naphthamide disodium salt;
- (C) The nondiffusible acid dye-releasing coupler releasing a diffusible magenta acid dye is selected from the group consisting of
- (1) 1-phenyl - 3 - (3,5 - disulfobenzamido)-4-(2-hydroxy-4-n-pentadecylphenylazo) - 5 - pyrazolone dipotassium salt, and
  - (2) 1-phenyl-3-(3,5 - disulfobenzamido) - 4 - (4-octadecyloxyphenylazo) - 5 - pyrazolone disodium salt; and
- (D) the nondiffusible acid dye-releasing coupler releasing a diffusible cyan acid dye is selected from the group consisting of
- (1) 1-hydroxy - 4 - (3-octadecylcarbamylphenylthio) - N - ethyl - 3',5' - dicarboxy-2-naphthaniide, and
  - (2) 2 - (3,5 - disulfobenzamido)-5-methyl-4-(4-octadecyloxyphenylazo)phenol dipotassium salt.
12. A photographic element comprising at least two Color-Forming Units in layers sensitive to different regions of the visible spectrum, and a barrier layer separating each of said Color-Forming Units comprising a hydrophilic colloid containing a water-insoluble reactant capable of forming a water-insoluble salt with mercaptans; each of said Color-Forming Units comprising

- (1) a light-sensitive emulsion of a hydrophilic colloid and a silver halide,
- (2) a nondiffusible and non-color forming development inhibitor-releasing hydroquinone compound contiguous to said silver halide of said light-sensitive emulsion that releases a diffusible mercaptan development inhibitor on reaction with oxidized developing agent of a photographic alkaline color developing solution containing an aromatic primary amino developing agent,
- (3) a developable emulsion of a hydrophilic colloid and a water-insoluble metal salt developable to substantial density without exposure to light with said color developing solution,
- (4) a nondiffusible acid-dye-releasing coupler contiguous to said water-insoluble metal salt of said developable emulsion that releases a diffusible acid dye on reaction with said oxidized developing agent; said acid dye-releasing coupler having a formula selected from the group consisting of

DYE-LINK-(COUP-BALL)<sub>n</sub>

and

BALL-LINK-(COUP-SOL)<sub>n</sub>

and said development inhibitor-releasing hydroquinone compound having the following general formula



wherein

- (1) DYE is a dye radical exhibiting selective absorption in the visible spectrum and containing an acidic solubilizing group,
- (2) LINK is a connecting radical selected from the group consisting of an azo radical, a mercuri radical, an oxy radical, an alkylidene radical, a monothio radical, a dithio radical and an azoxy radical,
- (3) —S— is a monothio connecting radical,
- (4) COUP is a photographic coupler radical selected from the group consisting of a 5-pyrazolone coupler radical, a phenolic coupler radical and an open-chain ketomethylene coupler radical, said COUP being substituted in the coupling position with one of said connecting radicals,
- (5) BALL is a photographically inert organic ballasting radical of such molecular size and configuration as to render said couplers and said hydroquinone compound nondiffusible,
- (6) SOL is selected from the group consisting of a hydrogen atom and an acidic solubilizing group when said developing agent contains an acidic solubilizing groups, and SOL is an acidic solubilizing group when said developing agent is free of an acidic solubilizing group,
- (7) n is an integer of 1 to 2 when said LINK is an alkylidene radical, and n is 1 when said LINK is a radical selected from the group consisting of an azo radical, a mercuri radical, an oxy radical, a monothio radical, a dithio radical and an azoxy radical,
- (8) RAD is a photographically inert diffusible radical that forms a mercaptan with said monothio connecting radical,
- (9) R is selected from the group consisting of a hydrogen atom and an alkaline splittable acyl masking group, and
- (10) R<sub>1</sub> is selected from the group consisting of a hydrogen atom and an alkaline splittable acyl masking group.

13. A photographic element as described in claim 12 wherein the developable emulsion is an emulsion of a hydrophilic colloid and a silver halide that is fogged so that it can be developed to substantial density without exposure to light with a photographic alkaline color developing solution containing an aromatic primary amino developing agent.

14. A photographic element as described in claim 12 wherein the developable emulsion is an emulsion of a hydrophilic colloid and a silver halide containing physical development nuclei.

15. A photographic element comprising a photographic support, three Color-Forming Units in layers sensitive to red, green and blue light respectively superposed on said support, and a barrier layer separating each of said Color-Forming Units comprising a hydrophilic colloid containing a silver halide; each of said Color-Forming Units comprising

(1) a light-sensitive emulsion layer of a hydrophilic colloid and a silver halide,

(2) a nondiffusible and non-color forming development inhibitor-releasing hydroquinone compound contiguous to said silver halide of said light-sensitive emulsion layer that releases a diffusible mercaptan development inhibitor on reaction with oxidized color developing agent of a photographic alkaline color developing solution containing an aromatic primary amino developing agent,

(3) a developable emulsion layer of a hydrophilic colloid and a water-insoluble silver salt developable to substantial density without exposure to light with said color developing solution, and

(4) a nondiffusible acid dye-releasing coupler capable of forming a diffusible acid dye contiguous to said water-insoluble silver salt of said developable emulsion layer on reaction with said oxidized developing agent, said acid dye-releasing coupler releasing a diffusible yellow acid dye when said light-sensitive emulsion layer is sensitive to blue light, a diffusible magenta dye when said light-sensitive emulsion layer is sensitive to green light and a diffusible cyan dye when said light-sensitive emulsion layer is sensitive to red light;

said acid dye-releasing coupler having a formula selected from the group consisting of

DYE-LINK-(COUP-BALL)<sub>n</sub>

and

BALL-LINK-(COUP-SOL)<sub>n</sub>

and said development inhibitor-releasing hydroquinone compound having the general formula



65 wherein

- (1) DYE is a dye radical exhibiting selective absorption in the visible spectrum and containing an acidic solubilizing group,
- (2) LINK is a connecting radical selected from the group consisting of an azo radical, a mercuri radical, an oxy radical, an alkylidene radical, a monothio radical, a dithio radical and an azoxy radical,
- (3) —S— is a monothio connecting radical,
- (4) COUP is a photographic coupler radical selected from the group consisting of a 5-pyrazolone coupler

radical, a phenolic coupler radical and an open-chain ketomethylene coupler radical, said COUP being substituted in the coupling position with one of said connecting radicals,

(5) BALL is a photographically inert organic ballasting radical of such molecular size and configuration as to render said couplers and said hydroquinone compound nondiffusible,

(6) SOL is selected from the group consisting of a hydrogen atom and an acidic solubilizing group when said developing agent contains an acidic solubilizing group, and SOL is an acidic solubilizing group when developing agent is free of an acidic solubilizing group,

(7) n is an integer of 1 to 2 when said LINK is an alkylidene radical, and n is 1 when said LINK is a radical selected from the group consisting of an azo radical, a mercuri radical, an oxy radical, a monothio radical, a dithio radical and an azoxy radical,

(8) RAD is a photographically inert diffusible radical that forms a mercaptan with said monothio connecting radical,

(9) R is selected from the group consisting of a hydrogen atom and an alkaline splittable acyl masking group, and

(10) R<sub>1</sub> is selected from the group consisting of a hydrogen atom and an alkaline splittable acyl masking group.

16. A photographic element as described in claim 15 wherein the development inhibitor-releasing hydroquinone compound is selected from the group consisting of

(1) 2-[4-[3-(4-tert-amyl-x-sulfophenoxy)benzamido]-phenylethyl] - x-(1-phenyl-5-tetrazolylthio)hydroquinone sodium salt,

(2) 5-[4-(3,5-disulfobenzamido)phenethyl]-2-methyl-3-(1-phenyl-5-tetrazolylthio)hydroquinone disodium salt,

(3) 2-[4-[2,4-di-tert-amylphenoxy]-5-(3,5-disulfobenzamido)-benzamido]phenylethyl] - x-(1-phenyl-5-tetrazolylthio)hydroquinone disodium salt dihydrate,

(4) 2-[4-[3-(4-tert-amyl-x-sulfophenoxy)benzamido]-phenethyl] - x-(1-phenyl-5-tetrazolylthio)hydroquinone diacetate sodium salt dihydrate,

(5) 2-[4-(3,5-disulfobenzamido)phenethyl]-x-(1-phenyl-5-tetrazolylthio)-hydroquinone disodium salt dihydrate

(6) 2-[4-(3,5-disulfobenzamido)phenethyl]-x-(2-benzoxazolylthio)-hydroquinone disodium salt dihydrate.

17. A photographic element comprising superposed on a photographic support three Color-Forming Units in layers sensitive to red, green and blue light respectively, the said Color-Forming Units sensitive to blue light being furthest from said support and being separated from the other of said Color-Forming Units by a barrier layer comprising a hydrophilic colloidal substrate containing a yellow filter material and a silver halide less sensitive to light than said Color-Forming Units, and the said Color-Forming Units sensitive to red and green light respectively being separated by a barrier layer comprising a hydrophilic colloidal substrate containing a silver halide less sensitive to light than said Color-Forming Units; each of said Color-Forming Units comprising

- (1) a light-sensitive emulsion layer of a hydrophilic colloid and a silver halide,
- (2) a nondiffusible and non-color forming development inhibitor-releasing hydroquinone compound contiguous to said silver halide of said light-sensitive emulsion layer that releases a diffusible mercaptan development inhibitor on reaction with oxidized color developing agent of a photographic alkaline color developing solution containing an aromatic primary amino developing agent,
- (3) a developable emulsion layer of a hydrophilic colloid and a water-insoluble silver salt developable to

substantial density without exposure to light with said developing agent and positioned closer to said support than said light-sensitive layer, and

(4) a nondiffusible acid dye-releasing coupler capable of forming a diffusible acid dye complementary to the color of the spectral sensitivity of the light-sensitive emulsion layer on reaction with said oxidized developing agent contiguous to said water-insoluble silver salt of said developable emulsion;

10 said acid dye-releasing coupler having the formula



and said development inhibitor-releasing hydroquinone compound having the formula



25 wherein

(1) LINK is a connecting radical selected from the group consisting of an azo radical, an oxy radical and a monothio radical,

(2) —S—is a monothio connecting radical,

(3) COUP is a photographic coupler radical selected from the group consisting of a 5-pyrazolone coupler radical, a phenolic coupler radical and an open-chain ketomethylene coupler radical, said COUP being substituted in the coupling position with one of said connecting radicals,

(4) BALL is a photographically inert organic ballasting radical of such molecular size and configuration as to render said couplers and said hydroquinone compound nondiffusible,

(5) SOL is selected from the group consisting of a hydrogen atom and an acidic solubilizing group when said developing agent contains an acidic solubilizing group, and SOL is an acidic solubilizing agent when said developing agent is free of an acidic solubilizing group,

(6) RAD is a photographically inert diffusible radical that forms a mercaptan with said monothio connecting radical,

(7) R is selected from the group consisting of a hydrogen atom and an alkaline splittable acyl masking group, and

(8) R<sub>1</sub> is selected from the group consisting of a hydrogen atom and an alkaline splittable acyl masking group.

18. A photographic element as described in claim 17 wherein the developable emulsion layer is an emulsion of a hydrophilic colloid and silver thiocyanate containing physical development nuclei.

19. A photographic element as described in claim 17 wherein the developable emulsion layer is an emulsion of a hydrophilic colloid and silver cyanide containing physical development nuclei.

20. A photographic element as described in claim 17 wherein the developable emulsion layer is an emulsion of a hydrophilic colloid and a silver halide fogged so that it can be developed to substantial density without exposure to light with a photographic alkaline color developing solution containing an aromatic primary amino developing agent.

21. A color photographic process for treating an exposed photographic element containing latent negative image regions and having superposed on a photographic support three Color-Forming Units in layers sensitive to red, green and blue light respectively, and a barrier layer separating each of said Color-Forming Units comprising

a hydrophilic colloid containing a silver halide, each of said Color-Forming Units comprising

- (1) a light-sensitive emulsion layer of a hydrophilic colloid and a silver halide,
- (2) a nondiffusible and non-color forming development inhibitor-releasing hydroquinone compound, contiguous to said silver halide of said light-sensitive emulsion layer, that releases a diffusible mercaptan development inhibitor on reaction with an oxidized color developing agent,
- (3) an emulsion layer of a hydrophilic colloid and a water-insoluble silver salt developable to substantial density with a color developing agent without exposure to light, and
- (4) a nondiffusible coupler capable of forming a non-diffusible dye contiguous to said water-insoluble silver salt of said developable emulsion layer on reaction with an oxidized color developing agent, said coupler forming a nondiffusible yellow dye when said light-sensitive emulsion layer is sensitive to blue light, a nondiffusible magenta dye when said light-sensitive emulsion layer is sensitive to green light and a non-diffusible cyan dye when said light sensitive emulsion layer is sensitive to red light; which comprises treating said exposed photographic element with a photographic alkaline color developing solution containing an aromatic primary amino developing agent so that in each of said Color-Forming Units, silver halide in said negative image regions of said light-sensitive emulsion layer is developed with said developing agent and said development inhibitor-releasing hydroquinone compound, contiguous to the silver halide, reacts with resulting oxidized developing agent to form a diffusible mercaptan development inhibitor in said negative image regions, said diffusible mercaptan development inhibitor thereafter diffusing to said developable emulsion layer and inhibiting development in regions corresponding to said negative image regions, said barrier layers preventing said diffusible mercaptan development inhibitor formed in one Color-Forming Unit from diffusing to another Color-Forming Unit by forming an insoluble silver salt with mercaptans diffusing to said barrier layers, said developable emulsion layer thereafter being developed with said developing agent and said non-diffusible dye-forming coupler contiguous to said water-insoluble silver salt in said developable emulsion layer reacting with resulting oxidized developing agent to form a nondiffusible dye in regions not inhibited against development by said mercaptan development inhibitor, and said nondiffusible dye remaining in said color-forming unit, from which unit is removed the developed silver and residual silver halide, said coupler having the following formula:

## COUP-BALL

and said development inhibitor-releasing hydroquinone compound having the formula



wherein

- (1) COUP is a photographic coupler radical selected from the group consisting of a 5-pyrazolone coupler radical, a phenolic coupler radical and an open-chain ketomethylene coupler radical, said COUP being substituted in the coupling position with a radical selected from the group consisting of hydrogen,

halogen, a sulfonic acid radical, an azo radical, a mercuri radical, an oxy radical, an alkylidene radical, a monothio radical, a dithio radical and an azoxy radical,

- (2) BALL is photographically inert organic ballasting radical of such molecular size and configuration as to render said couplers and said hydroquinone compound nondiffusible.
  - (3) —S— is a monothio connecting radical,
  - (4) SOL is selected from the group consisting of a hydrogen atom and a acidic solubilizing group when said developing agent contains an acidic solubilizing group, and SOL is an acidic solubilizing group when said developing agent is free of an acidic solubilizing group,
  - (5) RAD is a photographically inert diffusible radical that forms a mercaptan with said monothio connecting radical,
  - (6) R is selected from the group consisting of a hydrogen atom and an alkaline splittable acyl masking group, and
  - (7) R<sub>1</sub> is selected from the group consisting of a hydrogen atom and an alkaline splittable acyl masking group.
22. A color photographic process for treating an exposed photographic element containing latent negative image regions and having at least two Color-Forming Units in layers sensitive to different regions of the visible spectrum and a barrier layer separating each of said Color-Forming Units comprising a hydrophilic colloid containing a water-insoluble reactant capable of forming a water-insoluble salt with mercaptans, each of said Color-Forming Units comprising

- (1) a light-sensitive emulsion of a hydrophilic colloid and a silver halide;
- (2) an emulsion of a hydrophilic colloid and a water-insoluble metal salt developable to substantial density with a color developing agent without exposure to light;
- (3) a nondiffusible dye forming coupler contiguous to said water-insoluble metal salt of said developable emulsion and which coupler forms an image dye on reaction with an oxidized color developing agent; which comprises treating said exposed photographic element with a photographic alkaline color developing solution containing an aromatic primary amino developing agent so that in each of said Color-Forming Units said silver halide in said negative image regions of said light-sensitive emulsion is developed with said developing agent in the presence of a nondiffusible and non-color forming thio-substituted hydroquinone that reacts with oxidized color developing agent to form diffusible mercaptan development inhibitor in said negative image regions, reacting said hydroquinone with resulting oxidized developing agent and forming diffusible mercaptan development inhibitor, said diffusible mercaptan development inhibitor thereafter diffusing to said developable emulsion and inhibiting development in regions corresponding to said negative image regions, said barrier layer preventing said diffusible mercaptan development inhibitor formed in one Color-Forming Unit from diffusing to another Color-Forming Unit by forming an insoluble salt with mercaptans diffusing to said barrier layer, said developable emulsion thereafter being developed with said developing agent in the presence of said image dye forming coupler that reacts with resulting oxidized developing agent to form a dye image in regions not inhibited against development by said mercaptan development inhibitor.

23. The color photographic process defined in claim 22 wherein said thio-substituted hydroquinone is selected from the group consisting of an x-(5-tetrazolylthio)hydroquinone and an x-(2-benzoxazolyl) hydroquinone.

24. A photographic element comprising at least two Color-Forming Units in layers sensitive to different regions of the visible spectrum, and a barrier layer separating each of said Color-Forming Units comprising a hydrophilic colloid containing a water-insoluble reactant capable of forming a water-insoluble salt with mercaptans; each of said Color-Forming Units comprising

- (1) a light-sensitive emulsion of a hydrophilic colloid and a silver halide,
- (2) a nondiffusible and non-color forming development inhibitor-releasing thio-substituted hydroquinone contiguous to said silver halide of said light-sensitive emulsion that releases a diffusible mercaptan development inhibitor on reaction with oxidized developing agent of a photographic alkaline color developing solution containing an aromatic primary amino developing agent,
- (3) a developable emulsion of a hydrophilic colloid and a water-insoluble metal salt developable to substan-

5

10

15

20

tial density without exposure to light with said color developing solution, and

- (4) a nondiffusible dye-releasing coupler contiguous to said water-insoluble metal salt of said developable emulsion that forms a dye image on reaction with said oxidized developing agent.

25. A photographic element as defined in claim 24 wherein said thio-substituted hydroquinone is selected from the group consisting of an x-(5-tetrazolylthio) hydroquinone and an x-(2-benzoxazolyl) hydroquinone.

#### References Cited

##### UNITED STATES PATENTS

|           |        |                 |       |
|-----------|--------|-----------------|-------|
| 3,043,690 | 7/1962 | Green et al.    | 96—66 |
| 3,148,062 | 9/1964 | Whitmore et al. | 96—3  |
| 3,243,294 | 3/1966 | Barr            | 96—3  |

NORMAN G. TORCHIN, *Primary Examiner.*

J. TRAVIS BROWN, *Examiner.*